# EUROPEAN PATENT APPLICATION

(11) **EP 4 786 621 A1**
(43) Date of publication of application: **05.08.2026**
(21) Application number: 24872561.6
(22) Date of filing: 27.09.2024
(51) Int. Cl.: C22C 38/00, C21D 8/12, H01F 1/147, H01F 27/245, H01F 41/02, C21D 9/46, C22C 38/60

(54) **GRAIN-ORIENTED ELECTROMAGNETIC STEEL SHEET AND METHOD FOR PRODUCING GRAIN-ORIENTED ELECTROMAGNETIC STEEL SHEET**

(30) Priority: 27.09.2023 JP 2023166083
(71) Applicant: Nippon Steel Corporation, Tokyo 100-8071 (JP)
(72) Inventor: MATSUBARA, Ryo, Tokyo 100-8071 (JP); KAWAMURA, Yusuke, Tokyo 100-8071 (JP); HONMA, Rei, Tokyo 100-8071 (JP); SUZUMA, Toshiyuki, Tokyo 100-8071 (JP)
(74) Representative: Vossius & Partner Patentanwälte Rechtsanwälte mbB
(86) International application number: PCT/JP2024/034799
(87) International publication number: WO 2025/070780

(57) **Abstract**

A grain-oriented electrical steel sheet has plural magnetic domain control treatment lines on a surface thereof. When imaginary lines are set with a spacing of 5 mm in an evaluation region, in at least one of the imaginary lines, a standard deviation of distances of magnetic domain control points which are intersection points between the imaginary lines and the magnetic domain control treatment lines is 1.25 mm or more, and an average value of spacing of magnetic domain walls measured along the imaginary line is 600 µm or less.

## Description

### TECHNICAL FIELD

The present disclosure relates to a grain-oriented electrical steel sheet and a method for manufacturing a grain-oriented electrical steel sheet.

Priority is claimed on Japanese Patent Application No. 2023-166083, filed September 27, 2023, the content of which is incorporated herein by reference.

### BACKGROUND ART

The grain-oriented electrical steel sheet is a steel sheet containing 7 mass% or less of Si and having a secondary recrystallization structure in which secondary recrystallized grains are accumulated in a {110}<001> orientation (Goss orientation) in which an easy axis of magnetization <001> is oriented in a rolling direction. Grain-oriented electrical steel sheets are mainly used as iron cores of power transformers. Grain-oriented electrical steel sheets are required to reduce energy loss (iron loss).

A technique of narrowing a spacing of magnetic domain walls of a grain-oriented electrical steel sheet (magnetic domain refinement technique by magnetic domain control treatment) for reducing iron loss has been known for a long time. The spacing of magnetic domain walls can be narrowed by irradiating the surface of the grain-oriented electrical steel sheet with a laser or an electron beam in a direction intersecting the rolling direction to introduce a thermal strain. The spacing of magnetic domain walls can also be narrowed by forming a groove in the direction intersecting the rolling direction on the surface of the grain-oriented electrical steel sheet. Examples of a method of forming the groove include a method of irradiating with a laser or an electron beam, a method by mechanical processing such as gear, and a method by chemical processing such as etching.

In recent years, in order to provide a grain-oriented electrical steel sheet having good iron loss characteristics, various improved techniques related to magnetic domain refinement have been proposed (see, for example, Patent Documents 1 to 3.).

### Citation List

### Patent Documents

Patent Document 1: Japanese Unexamined Patent Application, First Publication No. 2012-57219
Patent Document 2: Japanese Unexamined Patent Application, First Publication No. 2012-12664
Patent Document 3: Japanese Unexamined Patent Application, First Publication No. 2012-57218

### SUMMARY OF INVENTION

### Technical Problem

When the magnetic domain control treatment is applied to the grain-oriented electrical steel sheet, the magnetostrictive characteristic of the grain-oriented electrical steel sheet changes depending on the flux closure domain. As a result, noise characteristics of the grain-oriented electrical steel sheet deteriorate. The noise characteristic is a degree of noise generated by an electrical product (for example, a transformer, a motor, and the like) manufactured using a grain-oriented electrical steel sheet as a material. Magnetostriction is a phenomenon in which an outer shape is slightly deformed when a ferromagnetic material is magnetized. When the grain-oriented electrical steel sheet is excited by alternating current, the magnitude of the magnetostriction changes with a change in the strength of magnetization, and thus vibration occurs. The magnitude of the magnetostriction is very small on the order of 10⁻⁶, but the magnetostriction generates vibration in the iron core, and the vibration propagates to an external structure such as a tank of a transformer to become noise. That is, the magnetic domain control treatment is effective for reducing iron loss of the grain-oriented electrical steel sheet, but deteriorates noise characteristics of the grain-oriented electrical steel sheet.

In recent years, there is an increasing demand for not only a reduction in iron loss but also a reduction in noise for grain-oriented electrical steel sheets. However, no magnetic domain refinement technique capable of sufficiently achieving both noise reduction and iron loss reduction has been proposed so far.

An object of the present disclosure is to provide a grain-oriented electrical steel sheet capable of achieving both iron loss reduction and noise reduction, and a manufacturing method therefore.

### Solution to Problem

The gist of the present disclosure is as follows.
(1) A grain-oriented electrical steel sheet according to an aspect of the present disclosure has plural magnetic domain control treatment lines on a surface thereof, wherein,
   when an evaluation region with a square shape where a length of each side is 50 mm and a side is parallel to a rolling direction of the grain-oriented electrical steel sheet is determined in the grain-oriented electrical steel sheet and when imaginary lines parallel to the rolling direction with a length of 50 mm are set with a spacing of 5 mm in the evaluation region,
   in at least one of the imaginary lines, a standard deviation of distances of magnetic domain control points which are intersection points between the imaginary lines and the magnetic domain control treatment lines is 1.25 mm or more, and an average value of spacing of magnetic domain walls measured along the imaginary line is 600 µm or less.
(2) Preferably, in the grain-oriented electrical steel sheet according to (1),
   in the imaginary lines where the standard deviation of the distances of the magnetic domain control points is 1.25 mm or more, the average value of the spacing of magnetic domain walls is 500 µm or less.
(3) A grain-oriented electrical steel sheet according to an aspect of the present disclosure has plural magnetic domain control treatment lines on a surface thereof, wherein,
   when an evaluation region with a square shape where a length of each side is 50 mm and a side is parallel to a rolling direction of the grain-oriented electrical steel sheet is determined in the grain-oriented electrical steel sheet and when imaginary lines parallel to the rolling direction with a length of 50 mm are set with a spacing of 5 mm in the evaluation region,
   in at least one of the imaginary lines, a standard deviation of distances of magnetic domain control points which are intersection points between the imaginary lines and the magnetic domain control treatment lines is 1.25 mm or more, and a maximum value of spacing of magnetic domain walls measured along the imaginary line is 1200 µm or less.
(4) Preferably, in the grain-oriented electrical steel sheet according to (3),
   in the imaginary lines where the standard deviation of the distances of the magnetic domain control points is 1.25 mm or more, the maximum value of the spacing of magnetic domain walls is 800 µm or less.
(5) Preferably, in the grain-oriented electrical steel sheet according to (1),
   in each of two or more of the imaginary lines, the standard deviation of the distances of the magnetic domain control points is 1.25 mm or more, and the average value of the spacing of magnetic domain walls is 600 µm or less.
(6) Preferably, in the grain-oriented electrical steel sheet according to (5),
   in each of two or more of the imaginary lines where the standard deviation of the distances of the magnetic domain control points is 1.25 mm or more, the average value of the spacing of magnetic domain walls is 500 µm or less.
(7) Preferably, in the grain-oriented electrical steel sheet according to (1) to (2) and (5) to (6),
   in at least one of the imaginary lines, the standard deviation of the distances of the magnetic domain control points which are intersection points between the imaginary lines and the magnetic domain control treatment lines is 2.50 mm or more, and the average value of the spacing of magnetic domain walls measured along the imaginary line is 600 µm or less.
(8) Preferably, in the grain-oriented electrical steel sheet according to (1) to (2) and (5) to (7),
   in the imaginary lines where the standard deviation of the distances of the magnetic domain control points is 2.50 mm or more, the average value of the spacing of magnetic domain walls is 500 µm or less.
(9) Preferably, in the grain-oriented electrical steel sheet according to (1) to (2) and (5) to (8),
   in at least one of the imaginary lines in the imaginary lines where the standard deviation of the distances of the magnetic domain control points is 1.25 mm or more, a number of grain boundary points which are intersection points between the imaginary lines and grain boundaries is 2 points or less.
(10) Preferably, in the grain-oriented electrical steel sheet according to (1) to (2) and (5) to (9), in each of two or more of the imaginary lines, the number of grain boundary points is 2 points or less.
(11) Preferably, in the grain-oriented electrical steel sheet according to (3),
   in each of two or more of the imaginary lines, the standard deviation of the distances of the magnetic domain control points is 1.25 mm or more, and the maximum value of the spacing of magnetic domain walls is 1200 µm or less.
(12) Preferably, in the grain-oriented electrical steel sheet according to (11),
   in each of two or more of the imaginary lines where the standard deviation of the distances of the magnetic domain control points is 1.25 mm or more, the maximum value of the spacing of magnetic domain walls is 800 µm or less.
(13) Preferably, in the grain-oriented electrical steel sheet according to (3) to (4) and (11) to (12),
   in at least one of the imaginary lines, the standard deviation of the distances of the magnetic domain control points which are intersection points between the imaginary lines and the magnetic domain control treatment lines is 2.50 mm or more, and the maximum value of the spacing of magnetic domain walls measured along the imaginary line is 1200 µm or less.
(14) Preferably, in the grain-oriented electrical steel sheet according to (3) to (4) and (11) to (13),
   in the imaginary lines where the standard deviation of the distances of the magnetic domain control points is 2.50 mm or more, the maximum value of the spacing of magnetic domain walls is 800 µm or less.
(15) Preferably, in the grain-oriented electrical steel sheet according to (3) to (4) and (11) to (14),
   in at least one of the imaginary lines in the imaginary lines where the standard deviation of the distances of the magnetic domain control points is 1.25 mm or more, a number of grain boundary points which are intersection points between the imaginary lines and grain boundaries is 2 points or less.
(16) Preferably, in the grain-oriented electrical steel sheet according to (3) to (4) and (11) to (15), in each of two or more of the imaginary lines, the number of grain boundary points is 2 points or less.
(17) Preferably, in the grain-oriented electrical steel sheet according to any one of (1) to (16), the magnetic domain control treatment lines are thermal strain.
(18) Preferably, in the grain-oriented electrical steel sheet according to any one of (1) to (17), the magnetic domain control treatment lines are grooves.
(19) Preferably, in the grain-oriented electrical steel sheet according to any one of (1) to (18), in at least one of the imaginary lines, the standard deviation of the distances is less than 1.25mm.
(20) A method for manufacturing a grain-oriented electrical steel sheet according to another aspect of the present disclosure includes:
   a step of acquiring a magnetic domain image of an original sheet of a grain-oriented electrical steel sheet;
   a step of determining a magnetic domain control treatment region based on a distribution of spacing of magnetic domain walls in the magnetic domain image; and
   a step of applying a magnetic domain control treatment to the magnetic domain control treatment region determined based on the distribution of the spacing of magnetic domain walls; wherein,
   when an evaluation region with a square shape where a length of each side is 50 mm and a side is parallel to a rolling direction of the grain-oriented electrical steel sheet is determined in the grain-oriented electrical steel sheet and when imaginary lines parallel to the rolling direction with a length of 50 mm are set with a spacing of 5 mm in the evaluation region,
   in at least one of the imaginary lines, a standard deviation of distances of magnetic domain control points which are intersection points between the imaginary lines and the magnetic domain control treatment lines formed by the magnetic domain control treatment is controlled to 1.25 mm or more.
(21) Preferably, in the method for manufacturing the grain-oriented electrical steel sheet according to (20), a region where the spacing of magnetic domain walls is a predetermined value or more is set as the magnetic domain control treatment region.
(22) Preferably, in the method for manufacturing a grain-oriented electrical steel sheet according to (20) or (21), a distribution of the spacing of magnetic domain walls is derived from the magnetic domain image using a two-dimensional Fourier transform.
(23) Preferably, in the method for manufacturing a grain-oriented electrical steel sheet according to any one of (20) to (22), the magnetic domain control treatment is applied by irradiation with a laser or an electron beam.

### Advantageous Effects of Invention

According to the above aspects of the present disclosure, it is possible to provide a grain-oriented electrical steel sheet capable of achieving both iron loss reduction and noise reduction, and a method for manufacturing the same.

### BRIEF DESCRIPTION OF DRAWINGS

[FIG. 1] A plan view of a grain-oriented electrical steel sheet according to an embodiment of the present disclosure.
[FIG. 2] A plan view of a normal grain-oriented electrical steel sheet.
[FIG. 3A] A schema illustrating an example of distribution of the spacing of magnetic domain walls of a grain-oriented electrical steel sheet before a magnetic domain control treatment.
[FIG. 3B] A schema illustrating an example of distribution of the spacing of magnetic domain walls of a grain-oriented electrical steel sheet after a magnetic domain control treatment.
[FIG. 3C] A schema illustrating a difference between FIGS. 3A and 3B.
[FIG. 4] A graph illustrating a relationship between a spacing of magnetic domain walls before a magnetic domain control treatment and a spacing of magnetic domain walls after the magnetic domain control treatment.
[FIG. 5] A block diagram illustrating an example of a hardware constitution of the image acquisition device.
[FIG. 6] A block diagram illustrating an example of a hardware constitution of an analysis device.
[FIG. 7] A schematic diagram illustrating an example of a constitution of a laser irradiation device.
[FIG. 8] A flowchart illustrating a method for manufacturing a grain-oriented electrical steel sheet according to an embodiment of the present disclosure.
[FIG. 9] A schematic view showing a method of cutting out a plurality of partial regions from a magnetic domain image of a grain-oriented electrical steel sheet.
[FIG. 10] An example of a plurality of partial Fourier images obtained by applying two-dimensional Fourier transform to each of a plurality of partial regions cut out from a magnetic domain image of a grain-oriented electrical steel sheet.
[FIG. 11] A plan view of an original sheet of a grain-oriented electrical steel sheet.
[FIG. 12] A schematic view showing a method of measuring an average value or a maximum value of spacing of magnetic domain walls along imaginary line.

### DESCRIPTION OF EMBODIMENTS

### (1. Grain-oriented electrical steel sheet 1)

The grain-oriented electrical steel sheet 1 according to the present embodiment has plural magnetic domain control treatment lines 11 on a surface thereof, wherein,
when an evaluation region with a square shape where a length of each side is 50 mm and a side is parallel to a rolling direction RD of the grain-oriented electrical steel sheet 1 is determined in the grain-oriented electrical steel sheet 1 and when first imaginary lines VL1 parallel to the rolling direction RD with a length of 50 mm are set with a spacing of 5 mm in the evaluation region,
in at least one of the first imaginary lines VL1, a standard deviation of distances of magnetic domain control points VP which are intersection points between the first imaginary lines VL1 and the magnetic domain control treatment lines 11 is 1.25 mm or more, and at least one of the following conditions is satisfied.
   (1) An average value of spacing of magnetic domain walls measured along the first imaginary line VL1 is 600 µm or less.
   (2) A maximum value of spacing of magnetic domain walls measured along the first imaginary line VL1 is 1200 µm or less.

### (Magnetic domain control treatment line 11)

A plurality of the magnetic domain control treatment lines 11 provided on the surface of the grain-oriented electrical steel sheet 1 have a function of refining a 180° magnetic domain. By refining the magnetic domain, the iron loss of the grain-oriented electrical steel sheet 1 can be reduced. The magnetic domain is a collection of magnetic dipoles existing inside a ferromagnetic material, and is a small region where magnetic moments are aligned in one direction. The 180° magnetic domain is a magnetic domain in which the magnetization direction is the <100> orientation of the crystal and which is sandwiched between two 180° magnetic domain walls substantially parallel to the rolling direction RD. A distance (magnetic domain wall interval) between adjacent magnetic domain walls of the 180° magnetic domain is referred to as a spacing of the 180° magnetic domain walls. Hereinafter, unless otherwise specified, the spacing of the 180° magnetic domain walls is simply referred to as "spacing of magnetic domain walls".

Suitable examples of the magnetic domain control treatment line 11 are the thermal strain and the groove. By refining the magnetic domain, the iron loss of the grain-oriented electrical steel sheet 1 can be suppressed. However, the magnetic domain control treatment line 11 changes the magnetostrictive characteristic of the grain-oriented electrical steel sheet 1 according to the flux closure domain. As a result, noise characteristics of the grain-oriented electrical steel sheet 1 deteriorate.

The magnetic domain control treatment line 11 is formed in a direction intersecting the rolling direction RD of the grain-oriented electrical steel sheet 1. In the general grain-oriented electrical steel sheet 1 as exemplified in FIG. 2, the magnetic domain control treatment line 11 is formed over the entire width of the grain-oriented electrical steel sheet 1. However, in the grain-oriented electrical steel sheet 1 according to the present embodiment as exemplified in FIG. 1, it is not essential to provide the magnetic domain control treatment line 11 over the entire width of the grain-oriented electrical steel sheet 1.

In the grain-oriented electrical steel sheet 1 illustrated in FIG. 1, the magnetic domain control treatment line 11 is a straight line. On the other hand, the magnetic domain control treatment line 11 may be a curve. The magnetic domain control treatment line 11 may have a shape having a straight line portion and a bent portion. The magnetic domain control treatment line 11 may be provided on one surface or both surfaces of the grain-oriented electrical steel sheet 1. When the magnetic domain control treatment line 11 is provided on both surfaces of the grain-oriented electrical steel sheet 1, various aspects of the grain-oriented electrical steel sheet 1 according to the present embodiment may be applied to at least one surface of the grain-oriented electrical steel sheet 1.

### (Evaluation region)

In the grain-oriented electrical steel sheet 1 according to the present embodiment, an evaluation region with a square shape where a length of each side is 50 mm and a side is parallel to a rolling direction RD of the grain-oriented electrical steel sheet 1 is determined in order to set the first imaginary lines VL1 explained below.

### (Imaginary lines (first imaginary lines) VL1 parallel to the rolling direction RD with a length of 50 mm)

In the grain-oriented electrical steel sheet 1 according to the present embodiment, the imaginary line is used for convenience in order to define a density of the magnetic domain control treatment lines 11. The imaginary lines are set inside the evaluation region with a spacing of 5 mm. FIG. 1 illustrates a state in which only one first imaginary lines VL1 is drawn as an example. In a case where a plurality of first imaginary lines VL1 is set, the required number of other first imaginary lines can be set in parallel to the first imaginary lines VL1 of FIG. 1. The length of the imaginary line is 50 mm. The imaginary line extends parallel to the rolling direction RD. An intersection point of the imaginary line and the magnetic domain control treatment line 11 is defined as a magnetic domain control point VP. The distance of the magnetic domain control points VP is an index of the density of the magnetic domain control treatment lines 11. Also, the imaginary lines are used as measurement positions for spacing of magnetic domain walls of the grain-oriented electrical steel sheet 1. Hereinafter, the imaginary line parallel to the rolling direction RD with a length of 50 mm is regarded as the first imaginary lines VL1.

### (Standard deviation of distances of magnetic domain control points VP)

In the grain-oriented electrical steel sheet 1 according to the present embodiment, in at least one of the first imaginary lines VL1, the standard deviation of the distances of magnetic domain control points VP is 1.25 mm or more. The distance d of magnetic domain control points VP is a distance between two magnetic domain control points VP adjacent to each other along the first imaginary line VL1. For example, the first imaginary lines VL1 of the grain-oriented electrical steel sheet 1 illustrated in FIG. 1 has eight magnetic domain control points VP. In a case where the standard deviation of the distances d1 to d7 of magnetic domain control points VP is 1.25 mm or more, the grain-oriented electrical steel sheet 1 in FIG. 1 satisfies the requirement of the present disclosure regarding the distances of magnetic domain control points VP.

As illustrated in FIG. 1, the grain-oriented electrical steel sheet 1 in which one or more first imaginary lines VL1 where the standard deviation of the distances of magnetic domain control points VP is 1.25 mm or more are arranged includes a region X where the magnetic domain control treatment line 11 is not provided.

Herein, the standard deviation of the distances of magnetic domain control points VP may change according to the position where the evaluation region and the first imaginary lines VL1 are arranged. In the grain-oriented electrical steel sheet 1 provided as an exemplary example in FIG. 1, it is also possible to position the evaluation region and the first imaginary lines VL1 such that the standard deviation of the distances of magnetic domain control points VP is less than 1.25 mm. However, it is considered that the grain-oriented electrical steel sheet 1 in which one or more first imaginary lines VL1 where the standard deviation of the distances of magnetic domain control points VP is 1.25 mm or more can be arranged at any place satisfies the requirement of the present disclosure regarding the distances of magnetic domain control points VP. Therefore, the grain-oriented electrical steel sheet 1 of FIG. 1 satisfies the requirement of the present disclosure regarding the distances of magnetic domain control points VP.

On the other hand, the grain-oriented electrical steel sheet 1 illustrated in FIG. 2 in which the plurality of magnetic domain control treatment lines 11 extending over the entire width of the grain-oriented electrical steel sheet 1 are arranged at equal intervals does not include the region X where the magnetic domain control treatment lines 11 are not provided. In the grain-oriented electrical steel sheet 1 of FIG. 2, a first imaginary lines VL1 where the standard deviation of the distances of magnetic domain control points VP is 1.25 mm or more cannot be arranged. Therefore, the grain-oriented electrical steel sheet 1 of FIG. 2 does not satisfy the requirement of the present disclosure regarding the distances of magnetic domain control points VP.

The standard deviation of the distances of magnetic domain control points VP is 1.25 mm or more, and an upper limit is not particularly limited. However, as necessary, the upper limit of the standard deviation of the distances of magnetic domain control points VP may be 23 mm.

### (Average value or Maximum value of spacing of magnetic domain walls measured along first imaginary line VL1)

The first imaginary lines VL1 where the standard deviation of the distances of magnetic domain control points VP is 1.25 mm or more further satisfies at least one of the following requirements.
(1) An average value of spacing of magnetic domain walls measured along the first imaginary line VL1 is 600 µm or less.
(2) A maximum value of spacing of magnetic domain walls measured along the first imaginary line VL1 is 1200 µm or less.

In the grain-oriented electrical steel sheet 1, both requirement (1) and requirement (2) may be satisfied. Specifically, in the first imaginary lines VL1 where the standard deviation of the distances of magnetic domain control points VP is 1.25 mm or more, the average value of the spacing of magnetic domain walls measured therealong may be 600 µm or less, and the maximum value may be 1200 µm or less. In the first imaginary lines VL1 where at least one of the requirement (1) and the requirement (2) is satisfied, the spacing of magnetic domain walls are controlled to a small value through the entire line.

It should be noted here that in the grain-oriented electrical steel sheet 1 according to the present embodiment, the distances of magnetic domain control points VP vary in the first imaginary lines VL1 which are the measurement position for the spacing of magnetic domain walls. The first imaginary lines VL1 which are the measurement position for the spacing of magnetic domain walls pass through the region X where the magnetic domain control treatment line 11 is not provided.

In general grain-oriented electrical steel sheet 1, the spacing of magnetic domain walls in the region X where the magnetic domain control treatment is not performed is wide. Thus, when the spacing of magnetic domain walls are measured along the first imaginary line VL1 which pass through the region X where the magnetic domain control treatment is not performed in general grain-oriented electrical steel sheet 1, the average value or the maximum value of the spacing of magnetic domain walls becomes extremely large. The skilled person in the art would try to make the region X where the magnetic domain control treatment is not performed as small as possible. However, the grain-oriented electrical steel sheet 1 according to the present embodiment, the average value and/or the maximum value of the spacing of magnetic domain walls which are measured along the first imaginary line VL1 where the standard deviation of the distances of magnetic domain control points VP is 1.25 mm or more are controlled into the above range.

The average value of the spacing of magnetic domain walls which is measured along the first imaginary line VL1 where the standard deviation of the distances of magnetic domain control points VP is 1.25 mm or more is further preferably 500 µm or less, 450 µm or less, 400 µm or less, 380 µm or less, 350 µm or less, or 300 µm or less. The maximum value of the spacing of magnetic domain walls which is measured along the first imaginary line VL1 is further preferably 1000 µm or less, 800 µm or less, 600 µm or less, 500 µm or less, 450 µm or less, or 400 µm or less.

### (Basic principle and effects)

The present inventors have found that, according to the grain-oriented electrical steel sheet 1 in which the first imaginary lines VL1
where the standard deviation of the distances of magnetic domain control points VP is 1.25 mm or more can be arranged and where the average value or the maximum value of the spacing of magnetic domain walls which is measured along the first imaginary line VL1 is small, both iron loss and noise can be reduced. This is because, in such a grain-oriented electrical steel sheet 1, the magnetic domain control treatment is applied only to a portion contributing to reduction of iron loss, and the magnetic domain control treatment line 11 is not provided in a portion where the magnetic domain control treatment is unnecessary. Hereinafter, the basic principle and effects of the present disclosure will be described with reference to FIGS. 3A to 3C and the like.

First, the present inventors compared the magnetic domain structure of the grain-oriented electrical steel sheet 1 before and after the magnetic domain control treatment. FIG. 3A shows an example of distribution of the spacing of magnetic domain walls of the grain-oriented electrical steel sheet 1 before the magnetic domain control treatment. FIG. 3B illustrates the distribution of the spacing of magnetic domain walls after the magnetic domain control treatment is performed on the surface of the grain-oriented electrical steel sheet 1 of FIG. 3A. The magnetic domain control treatment here is performed by applying continuous wave laser irradiation along a direction substantially perpendicular to the rolling direction RD. The distribution of the spacing of magnetic domain walls shown in FIGS. 3A and 3B is derived from the magnetic domain image of the grain-oriented electrical steel sheet 1 using two-dimensional Fourier transform described later.

FIG. 3C illustrates a difference between FIGS. 3A and 3B. FIG. 3C illustrates a region refined to a spacing of magnetic domain walls of 50 µm or more before and after the magnetic domain control treatment illustrated in FIGS. 3A and 3B. According to FIG. 3C, the region in which the spacing of magnetic domain walls is refined by the magnetic domain control treatment is visualized.

According to FIG. 3C, it can be seen that the region where the magnetic domain refinement of 50 µm or more has occurred by the magnetic domain control treatment is the dark color part of FIG. 3A, that is, the region where the spacing of magnetic domain walls is wide before the magnetic domain control treatment. In particular, it can be seen that the magnetic domain refinement effect remarkably appears in a region where the spacing of magnetic domain walls is originally about 500 µm or more. On the other hand, in the bright color part of FIG. 3A, that is, in the region where the spacing of magnetic domain walls is narrow before the magnetic domain control treatment, the effect of the magnetic domain control treatment hardly appears. The effect of the magnetic domain control treatment varies depending on the spacing of magnetic domain walls before the magnetic domain control treatment.

The present inventors investigated in more detail the relationship between the reduction amount of the spacing of magnetic domain walls caused by the magnetic domain control treatment and the spacing of magnetic domain walls before the magnetic domain control treatment. FIG. 4 shows the relationship between the spacing of magnetic domain walls before the magnetic domain control treatment and the spacing of magnetic domain walls before the magnetic domain control treatment at the same position. The magnetic domain control treatment was performed by laser irradiation. At the time of laser irradiation, the average irradiation energy density Ua (mJ/mm²) and the irradiation pitch PL (mm) were set to Ua = 1.5 mJ/mm² and PL = 4 mm, respectively.

According to FIG. 4, it can be seen that the magnetic domain refinement effect by the magnetic domain control treatment is less likely to appear in the region where the spacing of magnetic domain walls is narrow. In particular, in the region where the spacing of magnetic domain walls was about 500 µm or less, the spacing of magnetic domain walls were substantially the same before and after the magnetic domain control treatment. Therefore, it is considered that the effect of reducing the iron loss by the magnetic domain control treatment is large in a region where the spacing of magnetic domain walls before magnetic domain control is wide, but is not sufficiently obtained in a region where the spacing of magnetic domain walls before magnetic domain control is sufficiently narrow. It is considered that the magnetic domain control treatment line 11 formed in a region where the spacing of magnetic domain walls is narrow causes deterioration of noise characteristics due to the flux closure domain.

According to the above findings, in the conventional magnetic domain control treatment of the grain-oriented electrical steel sheet 1, the magnetic domain control is performed to a portion where the magnetic domain control is unnecessary, and this contributes to an increase in noise. In addition, it is found that it is extremely effective to preferentially perform the magnetic domain control treatment in a region having a wide spacing of magnetic domain walls in order to achieve both iron loss reduction and noise reduction. Magnetic domain control treatment in a region having a wide spacing of magnetic domain walls can reduce iron loss. In addition, by minimizing the magnetic domain control treatment in a region where the spacing of magnetic domain walls is narrow, deterioration of noise characteristics can be prevented.

In the grain-oriented electrical steel sheet 1 according to the present embodiment, the magnetic domain control treatment line 11 is not provided in a region where the spacing of magnetic domain walls was narrow before the magnetic domain control treatment. Therefore, the grain-oriented electrical steel sheet 1 according to the present embodiment includes the region X where the magnetic domain control treatment line 11 is not provided. In a case where the evaluation region and the first imaginary lines VL1 are set in the region X, the standard deviation of the distances of magnetic domain control points VP along the first imaginary line VL1 is 1.25 mm or more. By not providing the magnetic domain control treatment line 11, noise characteristics of the grain-oriented electrical steel sheet 1 according to the present embodiment are improved.

The region X where the magnetic domain control treatment line 11 is not provided is a region where the spacing of magnetic domain walls is narrow before the magnetic domain control treatment. Therefore, in the grain-oriented electrical steel sheet 1 according to the present embodiment, the spacing of magnetic domain walls is narrow even in the region X where the magnetic domain control treatment line 11 is not provided. In the grain-oriented electrical steel sheet 1 according to the present embodiment, the iron loss is not deteriorated in the region X where the magnetic domain control treatment line 11 is not provided.

In addition, in the grain-oriented electrical steel sheet 1 according to the present embodiment, the magnetic domain control treatment is performed on a region having a wide spacing of magnetic domain walls before the magnetic domain control treatment. Therefore, the iron loss of the grain-oriented electrical steel sheet 1 according to the present embodiment is reduced by the magnetic domain control treatment.

The most basic aspect of the grain-oriented electrical steel sheet 1 according to the present embodiment has been described above. Hereinafter, a more preferred aspect will be described.

(Number of first imaginary lines VL1 where standard deviation of distances of magnetic domain control points VP is 1.25 mm or more)
According to the examination results of the present inventors, in the original sheet 2 before the magnetic domain control treatment, regions having a narrow spacing of magnetic domain walls (regions not requiring the magnetic domain control treatment) were scattered on the entire surface of the original sheet 2. It is preferable to appropriately perform the magnetic domain control by avoiding all the regions with narrow spacing of magnetic domain walls scattered on the entire surface of the original sheet 2. Accordingly, also in the grain-oriented electrical steel sheet 1 after the magnetic domain control treatment, it is desirable that the regions X where the magnetic domain control treatment lines 11 are not provided are scattered on the entire surface.

Therefore, in the grain-oriented electrical steel sheet 1 according to the present embodiment, in a case where the first imaginary lines VL1 parallel to the rolling direction RD with a length of 50 mm is set at intervals of 5 mm inside the evaluation region, in each of two or more first imaginary lines VL1, it is preferable that the standard deviation of the distances of magnetic domain control points VP is 1.25 mm or more. That is, the grain-oriented electrical steel sheet 1 preferably includes the region X where the magnetic domain control treatment line 11 is not provided to such an extent that two or more first imaginary lines VL1 where the standard deviation of the distances of magnetic domain control points VP is 1.25 mm or more can be set. The number of the first imaginary lines VL1 where the standard deviation of the distances of magnetic domain control points VP is 1.25 mm or more is more preferably 3 or more, 4 or more, 5 or more, or 10 or more.

Moreover, from the viewpoint of further improving the iron loss, it is preferable that the spacing of magnetic domain walls is narrow in two or more first imaginary lines VL1 where the standard deviation of the distances of magnetic domain control points VP is 1.25 mm or more. Thus, it is preferable that at least one of the following requirements are satisfied in each of two or more first imaginary lines VL1.
(1) An average value of spacing of magnetic domain walls measured along the first imaginary line VL1 is 600 µm or less.
(2) A maximum value of spacing of magnetic domain walls measured along the first imaginary line VL1 is 1200 µm or less.

Moreover, in each of two or more first imaginary lines VL1 where the standard deviation of the distances of magnetic domain control points is 1.25 mm or more, the average value of the spacing of magnetic domain walls measured therealong is further preferably 500 µm or less, 450 µm or less, 400 µm or less, 380 µm or less, 350 µm or less, or 300 µm or less. In each of two or more first imaginary lines VL1 where the standard deviation of the distances of magnetic domain control points is 1.25 mm or more, the maximum value of the spacing of magnetic domain walls measured therealong is further preferably 800 µm or less, 600 µm or less, 500 µm or less, 450 µm or less, or 400 µm or less.

### (Aspect of magnetic domain control treatment line 11)

The type of the magnetic domain control treatment line 11 is not particularly limited, but suitable examples thereof are the thermal strain and/or the groove. The thermal strain can be formed using means such as laser irradiation, electron beam irradiation, and ion implantation. The groove can be formed using means such as laser irradiation, electron beam irradiation, and machining.

The thermal strain disappears by the stress relief annealing or the heat treatment according thereto. Therefore, when the grain-oriented electrical steel sheet 1 is subjected to a heat treatment, the magnetic domain control treatment line 11 is preferably a groove. On the other hand, since the thermal strain can be easily formed, when simplification of a manufacturing step is required, it is preferable to set the magnetic domain control treatment line 11 to the thermal strain. The grain-oriented electrical steel sheet 1 may include both the thermal strain and groove.

### (Standard deviation of distances of magnetic domain control points VP is 2.50 mm or more)

The grain-oriented electrical steel sheet 1 according to the present embodiment is characterized by selectively applying a magnetic domain control treatment to a region having a wide spacing of magnetic domain walls before magnetic domain control. In this case, a more remarkable effect can be obtained by applying the above treatment to a steel sheet having a coarse grain size than a steel sheet having a general grain size.

For example, in general, when the orientation development degree in the Goss orientation is to be increased in order to increase the magnetic flux density, the grain size tends to increase due to the manufacturing method. A steel sheet having such a coarse grain size has excellent magnetic flux density, but the iron loss tends to be high in a case where the magnetic domain control treatment is not performed because the grains are too large, and thus it is substantially necessary to perform the magnetic domain control. However, as described above, the conventional magnetic domain control treatment is effective in reducing the iron loss of the grain-oriented electrical steel sheet, but tends to deteriorate the noise characteristics of the grain-oriented electrical steel sheet.

On the other hand, when a magnetic domain control treatment is selectively performed on a steel sheet having a coarse grain size in a region having a wide spacing of magnetic domain walls before magnetic domain control as in the present embodiment, it is possible to obtain a grain-oriented electrical steel sheet capable of achieving both iron loss reduction and noise reduction in addition to excellent magnetic flux density.

When the magnetic domain control treatment unique to the present embodiment is performed on a steel sheet having a coarse grain size, the value of the standard deviation of the distances of magnetic domain control points VP particularly changes among the features described above because the steel sheet has a coarse grain size.

Specifically, it is preferable that the grain-oriented electrical steel sheet 1 according to the present embodiment satisfies the following feature. In at least one of the imaginary lines VL1, the standard deviation of the distances of magnetic domain control points VP which are intersection points between the imaginary lines VL1 and the magnetic domain control treatment lines 11 is preferably 2.50 mm or more, and the average value of the spacing of magnetic domain walls measured along the imaginary line VL1 is preferably 600 µm or less.

In addition, it is more preferable that the grain-oriented electrical steel sheet 1 according to the present embodiment satisfies the following feature. In each of two or more of the imaginary lines VL1, the standard deviation of the distances of magnetic domain control points VP which are intersection points between the imaginary lines VL1 and the magnetic domain control treatment lines 11 is preferably 2.50 mm or more, and the average value of the spacing of magnetic domain walls measured along the imaginary line VL1 is preferably 600 µm or less.

Moreover, it is preferable that the grain-oriented electrical steel sheet 1 according to the present embodiment satisfies the following feature. In at least one of the imaginary lines VL1, the standard deviation of the distances of magnetic domain control points VP which are intersection points between the imaginary lines VL1 and the magnetic domain control treatment lines 11 is preferably 2.50 mm or more, and the average value of the spacing of magnetic domain walls measured along the imaginary line VL1 is preferably 500 µm or less.

In addition, it is more preferable that the grain-oriented electrical steel sheet 1 according to the present embodiment satisfies the following feature. In each of two or more of the imaginary lines VL1, the standard deviation of the distances of magnetic domain control points VP which are intersection points between the imaginary lines VL1 and the magnetic domain control treatment lines 11 is preferably 2.50 mm or more, and the average value of the spacing of magnetic domain walls measured along the imaginary line VL1 is preferably 500 µm or less.

Moreover, it is preferable that the grain-oriented electrical steel sheet 1 according to the present embodiment satisfies the following feature. In at least one of the imaginary lines VL1, the standard deviation of the distances of magnetic domain control points VP which are intersection points between the imaginary lines VL1 and the magnetic domain control treatment lines 11 is preferably 2.50 mm or more, and the maximum value of the spacing of magnetic domain walls measured along the imaginary line VL1 is preferably 1200 µm or less.

In addition, it is more preferable that the grain-oriented electrical steel sheet 1 according to the present embodiment satisfies the following feature. In each of two or more of the imaginary lines VL1, the standard deviation of the distances of magnetic domain control points VP which are intersection points between the imaginary lines VL1 and the magnetic domain control treatment lines 11 is preferably 2.50 mm or more, and the maximum value of the spacing of magnetic domain walls measured along the imaginary line VL1 is preferably 1200 µm or less.

Moreover, it is preferable that the grain-oriented electrical steel sheet 1 according to the present embodiment satisfies the following feature. In at least one of the imaginary lines VL1, the standard deviation of the distances of magnetic domain control points VP which are intersection points between the imaginary lines VL1 and the magnetic domain control treatment lines 11 is preferably 2.50 mm or more, and the maximum value of the spacing of magnetic domain walls measured along the imaginary line VL1 is preferably 800 µm or less.

In addition, it is more preferable that the grain-oriented electrical steel sheet 1 according to the present embodiment satisfies the following feature. In each of two or more of the imaginary lines VL1, the standard deviation of the distances of magnetic domain control points VP which are intersection points between the imaginary lines VL1 and the magnetic domain control treatment lines 11 is preferably 2.50 mm or more, and the maximum value of the spacing of magnetic domain walls measured along the imaginary line VL1 is preferably 800 µm or less.

In a case where the magnetic domain control treatment unique to the present embodiment is performed on a steel sheet having a coarse grain size, the standard deviation of the distances of magnetic domain control points VP becomes the above specific value, and thus, it is unnecessary to specify the grain size of the grain-oriented electrical steel sheet 1 in the present embodiment. When the standard deviation of the distances of magnetic domain control points VP is 2.50 mm or more on the premise of satisfying that the standard deviation of the distances of magnetic domain control points VP is 1.25 mm or more by performing the magnetic domain control treatment unique to the present embodiment, it is possible to consider that the grain size of the grain-oriented electrical steel sheet 1 is coarse as compared to conventional steel sheet.

Herein, in the grain-oriented electrical steel sheet having a general grain size, the standard deviation of the distances of magnetic domain control points VP is usually less than 2.50 mm.

However, a method for judging whether a steel sheet has a coarse grain size may be to use the number of intersection points between imaginary lines and grain boundaries as an index. For instance, in the grain-oriented electrical steel sheet 1 according to the present embodiment, in at least one of the imaginary lines VL1 in the imaginary lines VL1 where the standard deviation of the distances of magnetic domain control points VP is 1.25 mm or more, a number of grain boundary points which are intersection points between the imaginary lines VL1 and grain boundaries may be 2 points or less.

In addition, in the grain-oriented electrical steel sheet 1 according to the present embodiment, in each of two or more of the imaginary lines VL1, the number of grain boundary points may be 2 points or less.

Herein, in the grain-oriented electrical steel sheet having a general grain size, the number of grain boundary points is approximately 3 to 10.

### (Number of imaginary lines VL1 where standard deviation of distances of magnetic domain control points VP is less than 1.25 mm)

Moreover, the grain-oriented electrical steel sheet 1 according to the present embodiment is characterized by selectively applying a magnetic domain control treatment to a region having a wide spacing of magnetic domain walls before magnetic domain control. In this case, in at least one of the imaginary lines VL1, the standard deviation of the distances of magnetic domain control points VP is 1.25 mm or more. On the other hand, in at least one of the imaginary lines VL1, the standard deviation of the distances of magnetic domain control points VP may be less than 1.25 mm.

Thus, in the grain-oriented electrical steel sheet 1 according to the present embodiment, in at least one of the imaginary lines VL1, the standard deviation of the distances of magnetic domain control points VP may be less than 1.25 mm.

Herein, in the grain-oriented electrical steel sheet 1 according to the present embodiment, the imaginary line VL1 where the standard deviation of the distances of magnetic domain control points VP may be less than 1.25 mm is not necessarily included in the evaluation region with the square shape where a length of each side is 50 mm and a side is parallel to the rolling direction of the grain-oriented electrical steel sheet. For instance, when the evaluation region is set to 20 areas, and when both of the imaginary line VL1 where the standard deviation of the distances of magnetic domain control points VP is 1.25 mm or more and the imaginary line VL1 where the standard deviation of the distances of magnetic domain control points VP is less than 1.25 mm are included in at least one of the evaluation regions, it can be considered that the magnetic domain control treatment is selectively applied to a region having a wide spacing of magnetic domain walls before magnetic domain control.

### (2. Manufacturing apparatus of grain-oriented electrical steel sheet 1)

Next, an example of a manufacturing apparatus of the grain-oriented electrical steel sheet 1 according to the present embodiment will be described. However, the manufacturing apparatus described below is merely exemplary. The grain-oriented electrical steel sheet 1 according to the present embodiment can be manufactured using an arbitrary device.

FIG. 5 illustrates an example of a hardware constitution of the image acquisition device 30 that acquires a magnetic domain image of the original sheet 2, that is, the grain-oriented electrical steel sheet 1 before the magnetic domain control treatment. The image acquisition device 30 includes a light source unit 31, a magneto-optical sensor (MO sensor 33), an image sensor 35, and a signal processing unit 37.

The light source unit 31 includes a light source including a light emitting diode (LED), and irradiates the MO sensor 33 with light having a uniform polarization plane.

The MO sensor 33 is a device that measures a magnetic domain structure of a magnetic material. The MO sensor 33 has an observed section on which a magnetic sample to be measured is placed. The light irradiated from the light source unit 31 passes through the inside of the MO sensor 33 and is reflected by the reflection layer. The reflected light passes through the inside of the MO sensor 33 again and is output to the outside of the MO sensor 33. When the original sheet 2 as a magnetic sample is placed on the observed section of the MO sensor 33, a leakage magnetic field corresponding to the direction of spontaneous magnetization of the original sheet 2 is generated inside the MO sensor 33. This leakage magnetic field rotates the polarization plane of the reflected light.

The image sensor 35 is a Complementary Metal-Oxide-Semiconductor (CMOS) image sensor. The image sensor 35 forms an image of the reflected light from the MO sensor 33 on the light receiving surface to perform photoelectric conversion, and outputs an analog signal after the photoelectric conversion to the signal processing unit 37. The distribution of the leakage magnetic field can be obtained by detecting the reflected light in which the polarization plane is rotated by the image sensor 35, and the magnetic domain structure of the original sheet 2 becomes clear.

The signal processing unit 37 includes an amplifier, an AD converter, a Digital Signal Processor (DSP), and the like. The analog signal output from the image sensor 35 is amplified by an amplifier. Then, the analog signal is converted into a digital signal by an AD converter. The digital signal is subjected to predetermined digital processing using a DSP to generate an image signal. The image signal generated by the signal processing unit 37 is output to the analysis device 40 (see FIG. 6) via a cable or by wireless communication.

FIG. 6 illustrates a hardware constitution of an analysis device 40 that analyzes the magnetic domain structure of the original sheet 2. The analysis device 40 is a computer device such as a personal computer (PC). The analysis device 40 includes a calculation unit 41, a memory 43, a display unit 45, an input unit 47, and a communication I/F 49.

The calculation unit 41 includes a Central Processing Unit (CPU). The calculation unit 41 analyzes the magnetic domain structure from the magnetic domain image of the original sheet 2 according to the program stored in the memory 43. Then, the calculation unit 41 determines a magnetic domain control treatment region 21 to which the magnetic domain control treatment is applied. The processing executed by the calculation unit 41 is described in detail later.

The memory 43 includes a Read Only Memory (ROM) and a Random Access Memory (RAM). The ROM stores programs executed by the CPU of the calculation unit 41 and data required for executing these programs. The program and data stored in the ROM are loaded into the RAM and executed.

The memory 43 may include a magnetic memory such as a hard disk drive (HDD) or an optical memory such as an optical disk. Alternatively, the memory 43 may be detachable from the analysis device 40 and store programs and data in a computer-readable recording medium. Alternatively, the memory 43 may receive the program executed by the calculation unit 41 from the network via the communication I/F 49.

The display unit 45 includes a display such as a liquid crystal display (LCD), a plasma display, or an organic electroluminescence (EL) display. The display unit 45 displays an image on the basis of the image signal output from the image acquisition device 30. In addition, the display unit 45 displays the analysis result of the magnetic domain structure by the calculation unit 41.

The input unit 47 includes an input device such as a mouse or a keyboard. The communication I/F 49 is an interface for transmitting and receiving data to and from an external device via a network such as a Local Area Network (LAN), a Wide Area Network (WAN), or the Internet.

Instead of general-purpose hardware such as a CPU, dedicated hardware specialized for analyzing a magnetic domain structure, such as an application specific integrated circuit (ASIC) or a Field Programmable Gate Array (FPGA), may be adopted as the calculation unit 41.

Note that FIGS. 5 and 6 illustrate a case where the image acquisition device 30 and the analysis device 40 are separate devices, but a system in which the image acquisition device 30 and the analysis device 40 are integrated may be adopted.

As means for introducing the thermal strain into the surface of the original sheet 2, known means such as laser irradiation, electron beam irradiation, and ion implantation can be adopted. As means for forming a groove on the surface of the original sheet 2, known means such as laser irradiation, electron beam irradiation, and machining can be adopted. Hereinafter, a constitution of the laser irradiation device 500 that introduces the thermal strain by laser irradiation will be described.

FIG. 7 illustrates a constitution of the laser irradiation device 500. The laser irradiation device 500 includes a polygon mirror 501, a light source device 503, a collimator 505, a condensing lens 507, a motor 509, a sensor 511, a control unit 513, and a sheet passing device 515.

The sheet passing device 515 passes the original sheet 2 in the rolling direction RD.

The polygon mirror 501 has, for example, a regular polygonal prism shape. A plurality of the plane mirrors is provided on each of a plurality of side surfaces constituting the polygon mirror 501 having a regular polygonal prism shape. The laser beam LB enters the plane mirror of the polygon mirror 501 in one direction (horizontal direction) from the light source device 503 via the collimator 505 and is reflected by the plane mirror.

The polygon mirror 501 is rotatable about the rotary shaft O1 by driving from the motor 509. The incident angle of the laser beam LB with respect to the plane mirror sequentially changes according to the rotation angle of the polygon mirror 501. As a result, the reflection direction of the laser beam LB is sequentially changed, and the surface of the original sheet 2 can be scanned. A Reference Number P in FIG. 7 represents an interval between the adjacent magnetic domain control treatment lines 11, that is, an irradiation pitch of the laser beam LB.

The light source device 503 outputs the laser beam LB by a predetermined irradiation system (for example, a continuous irradiation system or a pulse irradiation system) under the control of the control unit 513.

The condenser lens 507 is provided on the optical path of the laser beam LB reflected from the polygon mirror 501. The condenser lens 507 constitutes a condenser optical system having a predetermined focal distance. The laser beam LB reflected from the polygon mirror 501 is condensed on the surface of the original sheet 2 via the condenser lens 507, whereby the thermal strain is introduced into the surface of the original sheet 2.

The motor 509 is coupled to the polygon mirror 501. The motor 509 rotationally drives the polygon mirror 501 under the control of the control unit 513.

The sensor 511 is connected to a drive shaft of the motor 509. The sensor 511 detects a rotation angle of the polygon mirror 501 rotated by the motor 509. Furthermore, the sensor 511 outputs a signal (Hereinafter, the rotation angle signal is referred to as a rotation angle signal.) indicating the detected rotation angle to the control unit 513.

The control unit 513 includes a processor. The control unit 513 is connected to the light source device 503, the motor 509, the sensor 511, and the sheet passing device 515. The control unit 513 receives an input of a speed signal from the sheet passing device 515. Further, the control unit 513 outputs a signal instructing the motor 509 to rotationally drive the polygon mirror 501.

In addition, the control unit 513 controls on and off of the power of the laser beam LB output from the light source device 503 based on the stress introduction signal representing the magnetic domain control treatment region 21 and the rotation angle signal output from the sensor 511. When the laser irradiation device 500 is electrically connected to the analysis device 40, the stress introduction signal is input from the analysis device 40 to the laser irradiation device 500. The stress introduction signal may be input to the laser irradiation device 500 by an operator.

### (3. Method for manufacturing grain-oriented electrical steel sheet 1)

Next, a method for manufacturing the grain-oriented electrical steel sheet 1 according to the present embodiment will be described. According to the method for manufacturing a grain-oriented electrical steel sheet 1 according to the present embodiment, the grain-oriented electrical steel sheet 1 according to the present embodiment can be suitably manufactured. However, the manufacturing method described below is merely an example of a suitable manufacturing method of the grain-oriented electrical steel sheet 1, and does not limit the grain-oriented electrical steel sheet 1. For convenience of description, the manufacturing apparatus will be appropriately referred to in the description of the manufacturing method. However, the manufacturing apparatus mentioned below is merely a preferred example for carrying out the method for manufacturing the grain-oriented electrical steel sheet 1 according to the present embodiment.

As shown in the flowchart of FIG. 8, the method for manufacturing a grain-oriented electrical steel sheet 1 according to the present embodiment includes a step S62 of acquiring a magnetic domain image of an original sheet 2 of a grain-oriented electrical steel sheet 1, a step S64 of determining a magnetic domain control treatment region 21 based on distribution of the spacing of magnetic domain walls in the magnetic domain image, and a step S66 of applying the magnetic domain control treatment to the magnetic domain control treatment region 21 determined based on the distribution of the spacing of magnetic domain walls; wherein,
when an evaluation region with a square shape where a length of each side is 50 mm and a side is parallel to a rolling direction RD of the grain-oriented electrical steel sheet 1 is determined in the grain-oriented electrical steel sheet 1 and when first imaginary lines VL1 parallel to the rolling direction RD with a length of 50 mm are set with a spacing of 5 mm in the evaluation region,
in at least one of the first imaginary lines VL1, a standard deviation of distances of magnetic domain control points VP which are intersection points between the first imaginary lines VL1 and the magnetic domain control treatment lines 11 formed by the magnetic domain control treatment is controlled to 1.25 mm or more.

First, a magnetic domain image of the original sheet 2 is acquired (see S62 in FIG. 8). The original sheet 2 is the grain-oriented electrical steel sheet 1 before the magnetic domain control treatment is applied. The magnetic domain image can be acquired by, for example, the image acquisition device 30. Next, the distribution of the spacing of the 180° magnetic domain walls (spacing of magnetic domain walls) is derived from the magnetic domain image. The distribution of the spacing of magnetic domain walls in the original sheet 2 can be derived by using, for example, the calculation unit 41 of the analysis device 40.

Then, a region having a spacing of magnetic domain walls of a predetermined value or more (For example, about 500 µm or more) is determined as the magnetic domain control treatment region 21 (see S64 in FIG. 8). FIG. 11 shows an original sheet 2 of the grain-oriented electrical steel sheet 1 of FIG. 1. The shaded region in FIG. 11 is the magnetic domain control treatment region 21. The white region in FIG. 11 is the non-magnetic domain control treatment region 22. The spacing of magnetic domain walls of the magnetic domain control treatment region 21 is a predetermined value or more, and the spacing of magnetic domain walls of the non-magnetic domain control treatment region 22 is less than a predetermined value.

The magnetic domain control treatment region 21 may be determined by visually observing the magnetic domain image displayed on the display unit 45 by the operator, and a stress introduction signal representing the magnetic domain control treatment region 21 may be input to the laser irradiation device 500.

Next, the magnetic domain control treatment is preferentially performed on the magnetic domain control treatment region 21 (see S66 in FIG. 8). Preferably, the magnetic domain control treatment is performed only on the magnetic domain control treatment region 21. When the magnetic domain control treatment line 11 is a thermal strain, the magnetic domain control treatment may be executed by irradiation of the laser beam LB by the laser irradiation device 500, or other means such as ion implantation or electron beam irradiation may be adopted. When the magnetic domain control treatment line 11 is a groove, the magnetic domain control treatment may be executed using a tool for machining.

An example of a method for determining the magnetic domain control treatment region 21 will be described in detail. The processing for specifying the magnetic domain control treatment region 21 is executed by, for example, the calculation unit 41 of the analysis device 40.

The calculation unit 41 derives the distribution of the spacing of magnetic domain walls of the original sheet 2 using, for example, a line segment method or Fourier transform. Then, the calculation unit 41 determines a region where the spacing of magnetic domain walls is a predetermined value or more (For example, about 500 µm or more) as a portion to which the magnetic domain control treatment is preferentially applied.

In the line segment method, evaluation is performed by drawing a line segment perpendicular to the magnetic domain. The line segments are drawn at intervals of three lines per 1 cm in a direction parallel to the magnetic domain. A spacing of magnetic domain walls is derived based on a distance between the intersection points of 180° magnetic domain walls and line segments.

The Fourier transform is particularly effective as a means for analyzing a magnetic domain structure of a magnetic material having a periodic magnetic domain structure such as the grain-oriented electrical steel sheet 1 and the original sheet 2. Hereinafter, a method for deriving a distribution of a spacing of magnetic domain walls of the original sheet 2 is described using a short-term two-dimensional Fourier transform (Hereinafter, it is referred to as "ST2DFT".) obtained by expanding a short-term Fourier transform, which is one of signal processing methods that have been used for time-frequency analysis of audio signals for a long time, to a two-dimensional region.

An image (magnetic domain image) represented by an image signal acquired by the image acquisition device 30 is expressed as x (k, l) as a data column of two-dimensional coordinates (k-l coordinates). In the present embodiment, the magnetic domain image to be analyzed is an image binarized by two types of colors such as gray scale, or an image expressed by three or more gradations (multiple gradations).

In order to derive the distribution of the spacing of magnetic domain walls of the original sheet 2, the calculation unit 41 executes the following treatments of (A-1), (A-2), and (A-3).
(A-1) Treatment of cutting out a plurality of partial regions from magnetic domain image;
(A-2) Treatment of performing ST2DFT;
(A-3) Treatment of deriving distribution of spacing of magnetic domain walls.

Hereinafter, the treatment of A-1 to A-3 will be described in detail.

### (A-1) Treatment of cutting out a plurality of partial regions from magnetic domain image

In order to cut out a plurality of partial regions from a magnetic domain image and analyze each frequency structure, a window function Wa (k, l) of a rectangular window in which a range in the k direction set to 0 ≤ k ≤ Nₖ-1 and a range in the l direction set to 0 ≤ l ≤ Nₗ-1 is used (Nₖ and Nₗ are natural numbers). As the window function Wa (k, 1), a Hamming window, a Hanning window, a Blackman window, or the like can be applied.

When the observation position in the data column x (k, 1) of the magnetic domain image is expressed by an index (n, m), and the shift amounts of the window function Wa (k, l) in the k direction and the l direction are expressed as Sₖ and Sₗ, respectively (n, m, Sₖ, and Sₗ are integers.), a data column xₙₘ (k-nSₖ, l-mSₗ) of a partial region obtained by cutting out a range of nSₖ ≤ k ≤ nSₖ + Nₖ-1 and mSₗ ≤ l ≤ mSₗ + Nₗ-1 from the magnetic domain image is obtained as in Expression (1).
[Mathematical Formula 1] ${x}_{nm} \left(k-{nS}_{k},l-{mS}_{l}\right) = {W}_{a} \left(k-{nS}_{k},l-{mS}_{l}\right) x \left(k, l\right)$

FIG. 9 illustrates an example in which partial regions respectively corresponding to the observation positions (n, m) = (1, 1), (2, 2), (3, 3),..., and (P, Q) (P and Q are natural numbers) are cut out from the magnetic domain image G.

In the present embodiment, Nₖ and Nₗ that define the range of the window function Wa (k, 1) are parameters corresponding to the number of pixels in the k direction and the number of pixels in the l direction in the partial region, respectively.

### (A-2) Treatment of performing ST2DFT

When the data column of the partial region is defined as xₙₘ (n', m') = xₙₘ (k-nSₖ, l-mSₗ), and the two-dimensional Fourier transform is performed on xₙₘ (n', m'), a partial Fourier image X (fₖ, fₗ, n, m) corresponding to the partial region of the observation position (n, m) is obtained as in Expression (2).
[Mathematical Formula 2] $X \left({f}_{k}, {f}_{l}, n, m\right) = {\sum }_{n ′ = 0}^{{N}_{k} - 1} {\sum }_{m ′ = 0}^{{N}_{l} - 1} {x}_{nm} \left(n′,m′\right) exp \left\{-2πj\left(\frac{{f}_{k} n ′}{{N}_{k}}+\frac{{f}_{l} m ′}{{N}_{l}}\right)\right\}$

Here, fₖ and fₗ are space frequencies.

When the resolution of the space frequency fₖ is denoted by Δfₖ and the resolution of the space frequency fₗ is denoted by Δfₗ, Δfₖ and Δfₗ are defined as in Expression (3).
[Mathematical Formula 3] $\left\{\begin{matrix}Δ {f}_{k} = \frac{2}{{N}_{k} Δ k} \\ Δ {f}_{l} = \frac{2}{{N}_{l} Δ l}\end{matrix}\right.$ Δk and Δl are the space resolution in the k direction and the space resolution in the l direction in the magnetic domain image, respectively.

For example, when the two-dimensional Fourier transform is performed on the data column xₙₘ, (k-nSₖ, l-mSₗ) of each partial region illustrated in FIG. 9, a partial Fourier image X (fₖ, fₗ, n, m) is obtained for each observation position (n, m) as illustrated in FIG. 10.

### (A-3) Treatment of deriving distribution of spacing of magnetic domain walls

When the partial Fourier image X (fₖ, fₗ, n, m) is obtained, the coordinates (k component fₖ^{max} (n, m) and l component fₗ^{max} (n, m)) of the peak position of the spot of the partial Fourier image X (fₖ, fₗ, n, m) are obtained. Note that, regarding the derivation of the peak position, a region in the vicinity of k = 0 and l = 0 is a part that greatly depends on the contrast of the image, and thus is excluded.

Then, the distribution L (n, m) of the spacing of magnetic domain walls is derived as in Expression (4) from the resolution of the space frequency defined by Expression (3) and the peak position of the spot of the partial Fourier image.
[Mathematical Formula 4] $L \left(n, m\right) = \frac{1}{\sqrt{{\left(Δ{f}_{k}{f}_{k}^{max}\left(n, m\right)\right)}^{2} + {\left(Δ{f}_{l}{f}_{l}^{max}\left(n, m\right)\right)}^{2}}}$

As described above, by using ST2DFT, it is possible to quantitatively derive the distribution L (n, m) of the spacing of magnetic domain walls while maintaining the position information of the magnetic domain image. FIGS. 3A to 3C described above illustrate the analysis result of the spacing of magnetic domain walls derived by ST2DFT.

FIG. 11 is a plan view of an example of the original sheet 2. The original sheet 2 of FIG. 11 is a material of the grain-oriented electrical steel sheet 1 of FIG. 1. FIG. 11 illustrates a magnetic domain control treatment region 21 and a non-magnetic domain control treatment region 22 of the original sheet 2 which are specified based on the magnetic domain image. The magnetic domain control treatment region 21 is a region where the spacing of magnetic domain walls is a predetermined value or more. The non-magnetic domain control treatment region 22 is a region where the spacing of magnetic domain walls is less than a predetermined value. The magnetic domain control treatment is applied to a broken line provided inside the magnetic domain control treatment region 21 illustrated in FIG. 11. At this time, when an evaluation region with a square shape where a length of each side is 50 mm and a side is parallel to a rolling direction RD of the grain-oriented electrical steel sheet 1 is determined in the grain-oriented electrical steel sheet 1 and when first imaginary lines VL1 parallel to the rolling direction RD with a length of 50 mm are set with a spacing of 5 mm in the evaluation region, in at least one of the first imaginary lines VL1, a standard deviation of distances of intersection points between the first imaginary lines VL1 and the magnetic domain control treatment lines 11 along the first imaginary line VL1 is controlled to 1.25 mm or more. As a result, the grain-oriented electrical steel sheet 1 of FIG. 1 is obtained.

When the calculation unit 41 derives the distribution L(n, m) of the spacing of magnetic domain walls, the calculation unit 41 determines the region where the spacing of magnetic domain walls is the predetermined value or more as the magnetic domain control treatment region 21 (that is, a region to which the magnetic domain control treatment is applied). The control unit 513 of the laser irradiation device 500 performs control to turn on the power of the laser beam LB with respect to the magnetic domain control treatment region 21, and preferably, to turn off the power of the laser beam LB with respect to the non-magnetic domain control treatment region 22 (that is, a region other than the magnetic domain control treatment region 21). As a result, the magnetic domain control treatment line 11 is introduced into the magnetic domain control treatment region 21 of the original sheet 2. Further, in the non-magnetic domain control treatment region 22 of the original sheet 2, introduction of the magnetic domain control treatment line 11 is suppressed to a minimum.

The magnetic domain image of the grain-oriented electrical steel sheet 1 after the magnetic domain control treatment can also be obtained by the above-described procedure. In the magnetic domain image of the grain-oriented electrical steel sheet 1, the magnetic domain control treatment line 11 may be unclear. In this case, the observation conditions may be adjusted so that the magnetic domain control treatment line 11 can be clearly confirmed. For example, the magnetic domain control treatment line 11 can be clarified by applying a DC magnetic field along the sheet surface perpendicular direction (thickness direction) of the grain-oriented electrical steel sheet 1.

Although embodiments of the present disclosure have been described above, the present disclosure is not limited thereto, and can be appropriately modified without departing from the technical idea of the invention. Hereinafter, a more preferable example of the grain-oriented electrical steel sheet 1 according to the present embodiment and the method for manufacturing the same will be described. Unless otherwise specified, the preferred aspect described below is applicable to both the grain-oriented electrical steel sheet 1 and the method for manufacturing the same. As described later, the grain-oriented electrical steel sheet according to the present embodiment may have a forsterite film and/or an insulating coating on the surface of the base steel sheet.

Each will be described below. However, when the grain-oriented electrical steel sheet includes a base steel sheet and a forsterite film and/or an insulating coating, the following regulations regarding the chemical composition, the magnetic domain control treatment line, the magnetic domain control region, and the non-magnetic domain control treatment line are regulations regarding the base steel sheet. However, the provision regarding the sheet thickness is a provision regarding the entire grain-oriented electrical steel sheet including the base steel sheet, and the forsterite film and/or the insulating coating.

### (Chemical composition and sheet thickness)

The chemical compositions of the grain-oriented electrical steel sheet 1 and the original sheet 2 are not limited as long as they are equivalent to those of the known grain-oriented electrical steel sheet 1. For example, the grain-oriented electrical steel sheet 1 and the original sheet 2 can contain, as a chemical composition, Si: 2.500 to 7.000%, Mn: 0.00 to 1.000%, C: 0 to 0.085%, acid-soluble Al: 0 to 0.065%, N: 0 to 0.012%, Cr: 0 to 0.300%, Cu: 0 to 0.400%, P: 0 to 0.500%, Sn: 0 to 0.300%, Sb: 0 to 0.300%, Ni: 0 to 1.000%, S: 0 to 0.015%, Se: 0 to 0.015%, Bi: 0 to 0.020%, Nb: 0 to 0.030%, V: 0 to 0.030%, Mo: 0 to 0.030%, Ta: 0 to 0.030%, W: 0 to 0.030%, B: 0 to 0.080%, and Ti: 0 to 0.015% in mass%. The balance of the chemical composition includes Fe and impurities.

The sheet thicknesses of the grain-oriented electrical steel sheet 1 and the original sheet 2 are not limited, but are preferably 0.15 mm to 0.30 mm, for example. When the thickness is 0.30 mm or less, classical eddy-current loss can be suppressed, and iron loss can be further improved. On the other hand, when the sheet thickness is 0.15 mm or more, rolling efficiency can be improved to improve productivity.

### (Surface treatment)

The grain-oriented electrical steel sheet 1 and the original sheet 2 may have a forsterite film. The grain-oriented electrical steel sheet 1 and the original sheet 2 may have an insulating coating. The forsterite film and the insulating coating may be formed on one surface or both surfaces of the grain-oriented electrical steel sheet 1.

The forsterite film is, for example, an inorganic coating film containing magnesium silicate as a main component. The forsterite film is formed, for example, by a reaction between an annealing separator containing magnesia (MgO) applied to the surface of the base steel sheet and a component of the surface of the base steel sheet in final annealing. The forsterite film has, for example, a composition (more specifically, a composition containing Mg₂SiO₄ as a main component) derived from the components of the annealing separator and the base steel sheet. On the other hand, when an annealing separator mainly containing Al₂O₃ is used in final annealing, a forsterite film may not be formed.

The insulating coating has a function of applying electrical insulation properties and tension to the grain-oriented electrical steel sheet 1. The tension is applied to the grain-oriented electrical steel sheet 1 to facilitate magnetic domain wall movement in the grain-oriented electrical steel sheet 1, and thus, the iron loss of the grain-oriented electrical steel sheet 1 can be reduced. In addition, according to the insulating coating, various characteristics such as corrosion resistance, heat resistance, and slippage can be provided to the grain-oriented electrical steel sheet 1. The insulating coating may be, for example, a known coating formed by applying a coating solution containing phosphate and colloidal silica as main components to the surface of the forsterite film and baking the coating solution.

The insulating coating is preferably formed after the final annealing and after the magnetic domain control treatment. On the other hand, the insulating coating may be formed after the final annealing step and before the magnetic domain control treatment. When the insulating coating is formed before the magnetic domain control treatment, the insulating coating may be peeled off in the magnetic domain control treatment line 11. Therefore, it is preferable to form the insulating coating again on the magnetic domain control treatment line 11 after the magnetic domain control treatment.

### (Angle formed by magnetic domain control treatment line 11 and transverse direction TD)

The angle formed by the magnetic domain control treatment line 11 and the transverse direction TD is not particularly limited. The magnetic domain control treatment line 11 and the transverse direction TD may be substantially parallel. That is, the angle formed by the magnetic domain control treatment line 11 and the transverse direction TD may be substantially 0°. On the other hand, as illustrated in FIG. 1, the angle formed by the magnetic domain control treatment line 11 and the transverse direction TD may be more than 0°. For example, the angle formed by the magnetic domain control treatment line 11 and the transverse direction TD may be an arbitrary value within the range of 0° to 45°. The angle formed by the magnetic domain control treatment line 11 and the transverse direction TD may be 1° or more, 3° or more, or 5° or more. The angle formed by the magnetic domain control treatment line 11 and the transverse direction TD may be 40° or less, 35° or less, or 30° or less.

As illustrated in FIG. 1, the angles formed by all the magnetic domain control treatment lines 11 and the transverse direction TD may be the same. That is, all the magnetic domain control treatment lines 11 may extend in parallel to each other. On the other hand, the angle formed by the magnetic domain control treatment line 11 and the transverse direction TD may vary. That is, some or all of a plurality of the magnetic domain control treatment lines 11 may extend non-parallel to each other. The average value of the angles formed by the magnetic domain control treatment line 11 and the transverse direction TD may be 1° or more, 3° or more, or 5° or more. The average value of the angles formed by the magnetic domain control treatment line 11 and the transverse direction TD may be 40° or less, 35° or less, or 30° or less. The average value of the angles may be calculated by measuring an angle formed with the transverse direction TD at a plurality of positions with respect to one magnetic domain control treatment line, or by measuring an angle formed with the transverse direction TD by a plurality of magnetic domain control treatment lines at one point or a plurality of positions.

### (Interval P of magnetic domain control treatment)

For example, the interval P of magnetic domain control treatment such as the irradiation pitch P of laser beam LB illustrated in FIG. 7 is not particularly limited. As the interval P of the magnetic domain control treatment is smaller, the effect of reducing the iron loss is enhanced. On the other hand, as the interval P of the magnetic domain control treatment is larger, the noise characteristics is improved. The interval can be appropriately selected according to the characteristics required for the grain-oriented electrical steel sheet 1.

The intervals P at which the magnetic domain control treatment is performed correspond to distances between the magnetic domain control treatment lines 11 and imaginary lines therealong in the grain-oriented electrical steel sheet 1 according to the present embodiment. The imaginary line along the magnetic domain control treatment line 11 provided in the grain-oriented electrical steel sheet 1 is set over the entire width of the grain-oriented electrical steel sheet 1, and the intervals P of the magnetic domain control treatment are specified by measuring these intervals.

For example, the interval P of the magnetic domain control treatment may be 1.0 mm or more, 2.0 mm or more, 3.0 mm or more, or 5.0 mm or more. The interval P of the magnetic domain control treatment may be 10.0 mm or less, 9.0 mm or less, 8.0 mm or less, or 7.0 mm or less. Herein, the interval P of the magnetic domain control treatment is a value measured along the rolling direction RD.

In the grain-oriented electrical steel sheet 1 illustrated in FIG. 1, the interval P of the magnetic domain control treatment is constant. On the other hand, the interval P of the magnetic domain control treatment may vary. For example, the average value of the intervals P of the magnetic domain control treatment may be 1.0 mm or more, 2.0 mm or more, 3.0 mm or more, or 5.0 mm or more. The average value of the intervals P of the magnetic domain control treatment may be 10.0 mm or less, 9.0 mm or less, 8.0 mm or less, or 7.0 mm or less.

### (Magnitude of tensile stress introduced in thermal strain)

The magnetic domain control treatment line 11 may be due to a thermal strain. In the thermal strain, tensile stress is introduced. As the tensile stress is larger, the effect of improving the iron loss is enhanced. On the other hand, as the tensile stress is smaller, the noise characteristics are improved. Tensile stress according to characteristics required for the grain-oriented electrical steel sheet 1 can be appropriately selected.

The magnitude of the tensile stress is not particularly limited, but for example, in at least a part of the magnetic domain control treatment line 11, the tensile stress in an arbitrary direction is preferably 40 MPa or more, 60 MPa or more, or 80 MPa or more. When the tensile stress in at least one direction is 40 MPa or more, it is considered that the requirement that "the tensile stress in an arbitrary direction is 40 MPa or more" is satisfied. For example, in at least a part of the magnetic domain control treatment line 11, the tensile stress in an arbitrary direction is preferably 300 MPa or less, 200 MPa or less, 180 MPa or less, or 150 MPa or less. The tensile stress in an arbitrary direction in the magnetic domain control treatment line 11 may be uniform or may vary.

### (Depth and width of groove)

The magnetic domain control treatment line 11 may be a groove. As the depth and width of the groove are larger, the effect of improving the iron loss is enhanced. On the other hand, the noise characteristics are improved as the depth and width of the groove are smaller. The shape of the groove can be appropriately selected according to the characteristics required for the grain-oriented electrical steel sheet 1.

The depth of the groove is not particularly limited, but is preferably, for example, 5 µm to 50 µm. The depth of the groove may be 6 µm or more, 7 µm or more, or 10 µm or more. The depth of the groove may be 48 µm or less, 45 µm or less, or 40 µm or less.

The width of the groove (width at the opening part) is not particularly limited, but is preferably, for example, 10 µm to 300 µm. The width of the groove may be defined as 20 µm or more, 30 µm or more, or 50 µm or more. The width of the groove may be defined as 280 µm or less, 250 µm or less, or 200 µm or less. The depth and width of the groove may be uniform or may vary. In the case of variation, the average of the depths and widths of a plurality of the grooves is preferably in the above range.

### (Measurement method)

Hereinafter, a method for measuring various parameters of the grain-oriented electrical steel sheet 1 according to the present embodiment will be described. Note that measurement of any parameter is performed on a sample collected from the grain-oriented electrical steel sheet 1. For example, a rectangular sample having both sides of 100 mm (or 100 mm or more) in length can be cut out from the grain-oriented electrical steel sheet 1 and subjected to measurement. When the grain-oriented electrical steel sheet 1 is a coil, a sample may be collected from an arbitrary position of the coil. When the grain-oriented electrical steel sheet 1 is a component incorporated in an electrical product such as a transformer or a motor, a sample may be collected from any place of the component. When the size of the component is small, the length of one side of the sample may be less than 100 mm in so far as the length of one side of the sample is 50 mm or more. At that time, it is desirable to collect a sample by a method such as wire cutting in order to minimize the influence of mechanical strain or the like on the sample.

### (Method of identifying magnetic domain control treatment line 11)

When the magnetic domain control treatment line 11 is a groove, the magnetic domain control treatment line 11 can be visually identified. When the grain-oriented electrical steel sheet 1 has an insulating coating, the magnetic domain control treatment line 11 becomes visible by removing the insulating coating using a known peeling agent.

When the magnetic domain control treatment line 11 is a thermal strain, the magnetic domain control treatment line 11 may not be visually identified. In this case, for example, the magnetic domain image is photographed using the image acquisition device 30 as exemplified in FIG. 6. If necessary, a magnetic domain image is photographed while a DC magnetic field is applied along the rolling surface normal direction ND of the grain-oriented electrical steel sheet 1. The position of the thermal strain can be identified by observing the magnetic domain image.

### (Method for specifying rolling direction RD and transverse direction TD)

The rolling direction RD and the transverse direction TD of the grain-oriented electrical steel sheet 1 are specified by the following means.
(1) When the sample is cut out from the coil-shaped grain-oriented electrical steel sheet 1, the width direction of the coil is regarded as the transverse direction TD. A direction perpendicular to the transverse direction TD and the rolling surface normal direction ND is regarded as the rolling direction RD.
(2) When the sample is cut out from a part or the like of an electrical product, the rolling direction RD and the transverse direction TD are specified from rolling defects on the surface of the grain-oriented electrical steel sheet 1. The extending direction of the rolling defect is regarded as a rolling direction RD. A direction perpendicular to the rolling direction RD and the rolling surface normal direction ND is regarded as a transverse direction TD.
(3) When it is difficult to specify the rolling direction RD and the transverse direction TD from a rolling defect on the surface of the grain-oriented electrical steel sheet 1, the rolling direction RD and the transverse direction TD are specified from the crystal orientation of the grain-oriented electrical steel sheet 1. Specifically, the crystal orientation of the grain-oriented electrical steel sheet 1 to be evaluated is measured at a plurality of points. Then, the direction in which the deviation angle from the easy axis of magnetization <001> at which the angle formed by the crystal orientation at the measurement point with the rolling surface normal direction ND (sheet thickness direction) is the closest to the right angle is minimized is regarded as the rolling direction RD, and the direction perpendicular to the rolling direction RD and the rolling surface normal direction ND is regarded as the transverse direction TD.

### (Standard deviation of distances of magnetic domain control points VP)

The standard deviation of the distances of magnetic domain control points is calculated according to the following procedure. First, an evaluation region with a square shape where a length of each side is 50 mm and a side is parallel to the rolling direction RD of the grain-oriented electrical steel sheet 1 is determined in the grain-oriented electrical steel sheet 1. Then, first imaginary lines VL1 parallel to the rolling direction RD with a length of 50 mm are set with a spacing of 5 mm in the evaluation region on the surface of the grain-oriented electrical steel sheet 1. Next, a magnetic domain control point VP which is an intersection point of the first imaginary line VL1 and the magnetic domain control treatment line 11 is specified. The specification of the rolling direction RD and the magnetic domain control treatment line 11 is performed according to the above-described procedure. Then, the distances between the adjacent magnetic domain control points VP is measured, and the standard deviation of these measurement values is calculated.

The place where the evaluation region and the first imaginary line VL1 are set is not limited. The first imaginary line VL1 may be set at any place in which the first imaginary line VL1 where the standard deviation of the distances of magnetic domain control points VP falls within the range of the present disclosure can be set. For example, the first imaginary line VL1 may be set so as to pass through the region X where the magnetic domain control treatment line 11 is not provided. On the other hand, in a case where a place in which the first imaginary line VL1 where the standard deviation of the distances of magnetic domain control points VP falls within the range of the present disclosure can be set cannot be found, it is estimated that the requirements of the present disclosure are not satisfied.

### (Average value and maximum value of spacing of magnetic domain walls measured along first imaginary line VL1)

The average value and maximum value of the spacing of magnetic domain walls measured along the first imaginary line VL1 are calculated according to the following procedure.
(1) The magnetic domain image of the sample is photographed using the image acquisition device 30 as exemplified in FIG. 5.
(2) The first imaginary line VL1 used for measuring the standard deviation of the distances of magnetic domain control points VP is superimposed on the magnetic domain image.
(3) Plural imaginary lines perpendicularly intersecting the first imaginary line VL1 are set at intervals of 2 mm. Hereinafter, the plural imaginary lines perpendicularly intersecting the first imaginary line VL1 are referred to as second imaginary lines VL2. The length of each second imaginary line VL2 is 5 mm. The second imaginary line VL2 intersects with the first imaginary line VL1 at the center thereof.
(4) The number of magnetic domains included in each second imaginary line VL2 is measured. The value obtained by dividing the length of the second imaginary line VL2 by the number of magnetic domains included in this second imaginary line VL2 is regarded as the spacing of magnetic domain walls in the second imaginary line VL2.
(5) The average value and maximum value of the spacing of magnetic domain walls in the second imaginary line VL2 are calculated.

The method for measuring the spacing of magnetic domain walls in the second imaginary line VL2 is explained in detail below with reference to FIG. 12. FIG. 12 is a schematic view of magnetic domain image. In the magnetic domain image, a magnetic domain 601A and a magnetic domain 601B have a band shape. For clarity, adjacent magnetic domains are shown with different patterns in FIG. 12. Specifically, the magnetic domain 601A is hatched, and the magnetic domain 601B adjacent to the magnetic domain 601A is not hatched. The boundary between two adjacent magnetic domains 601A and 601B is a magnetic domain wall 602.

In FIG. 12, the first imaginary line VL1 and the second imaginary line VL2 are superimposed. The number of magnetic domains included in the upper second imaginary line VL2 in the figure is 11. Thus, the spacing of magnetic domain walls in the upper second imaginary line VL2 in the figure is considered to be 455 µm (=5000/11). The number of magnetic domains included in the lower second imaginary line VL2 in the figure is 23. Thus, the spacing of magnetic domain walls in the lower second imaginary line VL2 in the figure is considered to be 217 µm (=5000/23).

In each of plural first imaginary lines VL1, the average value and maximum value of the spacing of magnetic domain walls are determined according to the above-described procedure (1) to (5). In a case where the standard deviation of the distances of magnetic domain control points is 1.25 mm or more and the average value of the spacing of magnetic domain walls is 600 µm or less in at least one of the first imaginary lines VL1, the sample is regarded as the grain-oriented electrical steel sheet according to the present disclosure. Moreover, in a case where the standard deviation of the distances of magnetic domain control points is 1.25 mm or more and the maximum value of the spacing of magnetic domain walls is 1200 µm or less in at least one of the first imaginary lines VL1, the sample is also regarded as the grain-oriented electrical steel sheet according to the present disclosure. The number of the first imaginary lines VL1 satisfying the requirements of the present disclosure is preferably as large as possible.

### (Method for measuring chemical composition of original sheet 2 and grain-oriented electrical steel sheet 1)

The chemical compositions of the grain-oriented electrical steel sheet 1 and the original sheet 2 may be measured by a general analysis method of steel. For example, the chemical composition may be measured using inductively coupled plasma-atomic emission spectrometry (ICP-AES). Specifically, the chemical composition of the grain-oriented electrical steel sheet 1 and the original sheet 2 can be measured by acquiring a test piece from the center portion in the thickness direction of the sample, and measuring the test piece under a condition based on a calibration curve prepared in advance using ICPS-8100 manufactured by Shimadzu Corporation or the like (measuring device). The contents of C and S, which are difficult to measure by ICP-AES, may be measured using a combustion-infrared light absorption method. The content of N may be measured using an inert gas fusion-thermal conductivity method.

When a forsterite film and/or an insulating coating are/is formed on the grain-oriented electrical steel sheet 1 and the original sheet 2, chemical compositions of the grain-oriented electrical steel sheet 1 and the original sheet 2 may be analyzed after removing the forsterite film and/or the insulating coating from the grain-oriented electrical steel sheet 1 and the original sheet 2.

The forsterite film can be removed, for example, by immersing the sample in sulfuric acid followed by immersion in nitric acid. Conditions such as the temperature and concentration of sulfuric acid and nitric acid and the time for immersion are appropriately adjusted so that the base metal of the sample is not excessively dissolved. An example of conditions of the removal operation of the forsterite film is as follows. First, the sample is immersed in sulfuric acid having a concentration of 10% at 80°C for 3 minutes. Thereafter, the surface of the sample is washed with water using a waste cloth or the like to remove the sludge adhering to the surface. Thereafter, the sample is dried. Further, the sample is immersed in nitric acid having a concentration of 10% at room temperature while being stirred for about 5 seconds.

The insulating coating can be removed, for example, by immersing the sample in a sodium hydroxide solution and then immersing the sample in dilute sulfuric acid and nitric acid. Conditions such as the temperature and concentration of sodium hydroxide, dilute sulfuric acid, and nitric acid solution, and the time for immersion are appropriately adjusted so that the base metal of the sample is not excessively dissolved. An example of the conditions of the removal operation of the insulating coating is as follows. First, the sample is immersed in a sodium hydroxide solution having a concentration of 20% at 80°C for 15 minutes. Thereafter, the sample is dried. Then, the sample is immersed in diluted sulfuric acid having a concentration of 10% at 80°C for 4 minutes. Thereafter, the sludge adhering to the surface of the sample is removed with a waste cloth or the like. Further, the sample is immersed in nitric acid having a concentration of 10% at room temperature while being stirred for about 10 seconds.

### (Method of measuring angle formed by magnetic domain control treatment line 11 and transverse direction TD)

The angle formed by the magnetic domain control treatment line 11 and the transverse direction TD can be measured using a known angle measuring means after the magnetic domain control treatment line 11 and the transverse direction TD are specified by the above-described procedure.

### (Method of measuring interval P of magnetic domain control treatment)

The interval P of magnetic domain control treatment is obtained by identifying the magnetic domain control treatment line 11 and the rolling direction RD using the above procedure, by setting imaginary lines along the magnetic domain control treatment line 11, and then by measuring the interval of imaginary lines using a known length measuring procedure.

### (Method for measuring magnitude of tensile stress introduced in thermal strain)

The magnitude of the tensile stress introduced in the thermal strain is measured by the EBSD Wilkinson method and Cross Court manufactured by BLG Vantage. The EBSD Wilkinson method is described in detail in A.J.Wilkinson, et al. "High-resolution elastic strain measurement from electron backscatter diffraction patterns: New levels of sensitivity" Ultramicroscopy Vol 106, No. 4-5, March 2006, P. 307-313.

When the magnitude of the tensile stress introduced in the thermal strain is measured by the EBSD Wilkinson method and the Cross Court manufactured by BLG Vantage, first, the magnetic domain control treatment line 11 is specified by the above-described procedure. Next, the grain-oriented electrical steel sheet 1 is cut through the magnetic domain control treatment line 11 and perpendicularly to the magnetic domain control treatment line 11. This cut cross section is used as a measurement surface. The cross section of the magnetic domain control treatment line 11 included in the measurement surface is analyzed by the EBSD Wilkinson method and Cross Court manufactured by BLG Vantage, and a tensile stress component in an arbitrary direction is extracted and the magnitude thereof is measured. For example, it is possible to extract a tensile stress component in a rolling surface normal direction ND, a direction parallel to the magnetic domain control treatment line 11, and a direction perpendicular to the rolling surface normal direction ND and the magnetic domain control treatment line 11.

The number of measurement points is, for example, 10. When the tensile stress in an arbitrary direction is 40 MPa or more (that is, when the tensile stress in at least one direction is 40 MPa or more,) in at least one location of the grain-oriented electrical steel sheet 1, the maximum value of the tensile stress in an arbitrary direction in the magnetic domain control treatment line of the grain-oriented electrical steel sheet 1 is determined to be 40 MPa or more. The measurement of the tensile stress may be stopped when a measurement point at which the tensile stress in an arbitrary direction is 40 MPa or more is found.

### (Method of measuring depth and width of groove)

The depth and width of the groove can be measured by specifying the surface shape of the sample using a known three-dimensional measuring machine. When the grain-oriented electrical steel sheet 1 has an insulation coating, the insulating coating is removed by the above-described procedure, and then the three-dimensional measurement of the sample surface is performed.

### Examples

The effect of an aspect of the present disclosure will be described more specifically with reference to Examples. However, the conditions in Examples are merely one condition example adopted to confirm the enablement and effects of the present disclosure. The present disclosure is not limited to this one condition example. The present disclosure can adopt various conditions as long as the object of the present disclosure is achieved without departing from the gist of the present disclosure.

### (Example 1)

A grain-oriented electrical steel sheet (grain-oriented electrical steel sheet having general grain size) of the same lot having a sheet thickness of 0.23 mm which was classified as 23P085 in the table 2 of JIS C 2553:2019 "Cold-rolled grain-oriented electrical steel strip" was used as the original sheet. In these grain-oriented electrical steel sheets, for instance, the average temperature rising rate in a range from 1000 to 1200°C was 15°C/h during temperature rising process of final annealing. The original sheet was subjected to a magnetic domain control treatment under various conditions shown in Table 1. The noise and iron loss of the grain-oriented electrical steel sheets subjected to the magnetic domain control treatment obtained as a result were evaluated and are described in Table 2. In Table 2, values determined to be unacceptable are underlined.

Herein, the shapes of the magnetic domain control treatment lines were as follows. The shape applied to the sample is noted in the column "Remarks" of Table 1.

A: A magnetic domain control treatment line was formed in a region where the spacing of magnetic domain walls was the predetermined value or more as explained above.

B: A magnetic domain control treatment line was straight linearly formed over the entire width of the original sheet.

C: A magnetic domain control treatment line with an ordered broken linear shape was formed.

D: A magnetic domain control treatment line with a random broken linear shape was formed.

E: A magnetic domain control treatment line having an interval of 4 mm was formed only in a region within ±4 mm from the center of each crystal grain in the rolling direction RD. The radius of curvature of the steel sheet at the position where the grains were present during the final annealing was 250 mm.

The methods for evaluating the noise and iron loss were as follows. First, 180 grain-oriented electrical steel sheets having a sheet thickness of 0.23 mm were laminated to form a three-phase transformer core. The widths of the leg and the yoke of the three-phase transformer core were both 150 mm. The height and width of the outer shape of the three-phase transformer core were both 750 mm. Noise and iron loss of these three-phase transformer cores were measured. The measurement conditions were a frequency of 60 Hz and an excitation magnetic flux density of 1.7 T.

In measuring the noise, microphones were arranged at equal intervals at eight points around the transformer in which the three-phase transformer core was incorporated. The distance between the transformer and the microphone was 30 cm. The values obtained by correcting the A characteristics to the noise measurement results by the microphones and averaging the results are described in Table 2 as the noise evaluation results (unit: dBA) of the grain-oriented electrical steel sheets. An example in which the evaluation result of noise was 37.00 dBA or less was determined to be an example in which noise reduction was achieved. The noise evaluation result determined to be unacceptable was underlined.

The iron loss was obtained by measuring voltages and currents on the primary side and the secondary side with a power analyzer when excitation was performed at a frequency of 60 Hz and an excitation magnetic flux density of 1.7 T as described above. The obtained iron loss is described in Table 2 as an iron loss evaluation result (unit: W/kg) of the grain-oriented electrical steel sheet. An example in which the evaluation result of the iron loss was 1.10 W/kg or less was determined to be an example in which iron loss reduction was achieved. The noise evaluation result determined to be unacceptable was underlined.

Further, a standard deviation of distances of magnetic domain control points and spacing of magnetic domain walls were measured and described in Table 1. The measurement method was in principle according to the procedure described above. A rectangular sample having both sides of 100 mm in length was cut out from a three-phase transformer core for measuring noise and iron loss, and subjected to measurement.

In this rectangular sample, a square evaluation region having a side length of 50 mm and a side parallel to the rolling direction of the grain-oriented electrical steel sheet was set, and imaginary lines VL1 parallel to the rolling direction and having a length of 50 mm were set at intervals of 5 mm inside the evaluation region. The number of imaginary lines was nine.

In each of nine imaginary lines VL1, standard deviation of distances of magnetic domain control points was measured. The number of imaginary lines VL1 where the standard deviation of the distances of magnetic domain control points was 1.25 mm or more is noted in the column "Number of VL1 where standard deviation is 1.25 mm or more" of Table 1.

Moreover, in each of imaginary lines VL1 where the standard deviation of the distances of magnetic domain control points was 1.25 mm or more, an average spacing of magnetic domain walls and a maximum spacing of magnetic domain walls were measured. The number of imaginary lines VL1 where the average spacing of magnetic domain walls was 600 µm or less in the imaginary lines VL1 where the standard deviation of the distances of magnetic domain control points was 1.25 mm or more is noted in the column "Number of VL1 where average spacing of magnetic domain walls is 600 µm or less" of Table 1. The sample in which the number noted in the column "Number of VL1 where average spacing of magnetic domain walls is 600 µm or less" is 1 is regarded as the grain-oriented electrical steel sheet where the standard deviation of the distances of magnetic domain control points which are intersection points between the imaginary lines VL1 parallel to the rolling direction and having a length of 50 mm and the magnetic domain control treatment lines is 1.25 mm or more and the average value of the spacing of magnetic domain walls measured along the imaginary line VL1 is 600 µm or less. Moreover, the sample in which the number noted in the column "Number of VL1 where average spacing of magnetic domain walls is 600 µm or less" is 2 or more is regarded as the grain-oriented electrical steel sheet where the standard deviation of the distances of magnetic domain control points is 1.25 mm or more in two or more of the imaginary lines VL1 and the average value of the spacing of magnetic domain walls in two or more of the imaginary lines VL1 is 600 µm or less.

In the same way, the number of imaginary lines VL1 where the average spacing of magnetic domain walls was 500 µm or less in the imaginary lines VL1 where the standard deviation of the distances of magnetic domain control points was 1.25 mm or more is noted in the column "Number of VL1 where average spacing of magnetic domain walls is 500 µm or less" of Table 1. Moreover, the number of imaginary lines VL1 where the maximum spacing of magnetic domain walls was 1200 µm or less in the imaginary lines VL1 where the standard deviation of the distances of magnetic domain control points was 1.25 mm or more is noted in the column "Number of VL1 where maximum spacing of magnetic domain walls is 1200 µm or less" of Table 1. Moreover, the number of imaginary lines VL1 where the maximum spacing of magnetic domain walls was 800 µm or less in the imaginary lines VL1 where the standard deviation of the distances of magnetic domain control points was 1.25 mm or more is noted in the column "Number of VL1 where maximum spacing of magnetic domain walls is 800 µm or less" of Table 1.

Although not shown in the tables, in any imaginary lines VL1 where the standard deviation of the distances of magnetic domain control points VP was 1.25 mm or more, a number of grain boundary points which were intersection points between the imaginary lines VL1 and grain boundaries was 3 or more. Moreover, although not shown in the tables, in any imaginary lines VL1 where the standard deviation of the distances of magnetic domain control points VP was 1.25 mm or more, the standard deviation of the distances were less than 2.50 mm.

**[Table 1]**

| | NUMBER OF VL1 WHERE STANDARD DEVIATION IS 1.25 mm OR MORE | NUMBER OF VL1 WHERE AVERAGE SPACING OF MAGNETIC DOMAIN WALLS IS 600 *µ*m OR LESS | NUMBER OF VL1 WHERE AVERAGE SPACING OF MAGNETIC DOMAIN WALLS IS 500 *µ*m OR LESS | NUMBER OF VL1 WHERE MAXIMUM SPACING OF MAGNETIC DOMAIN WALLS IS 1200 *µ*m OR LESS | NUMBER OF VL1 WHERE MAXIMUM SPACING OF MAGNETIC DOMAIN WALLS IS 800 *µ*m OR LESS | TYPE OF MAGNETIC DOMAIN CONTROL TREATMENT LINE | REMARKS |
|---|---|---|---|---|---|---|---|
| 1 | 1 | 1 | 0 | 0 | 0 | THERMAL STRAIN | A |
| 2 | 1 | 1 | 0 | 0 | 0 | MIXED | A |
| 3 | 1 | 1 | 0 | 0 | 0 | GROOVE | A |
| 4 | 1 | 1 | 1 | 0 | 0 | THERMAL STRAIN | A |
| 5 | 1 | 0 | 0 | 1 | 0 | THERMAL STRAIN | A |
| 6 | 1 | 1 | 0 | 1 | 0 | THERMAL STRAIN | A |
| 7 | 1 | 0 | 0 | 1 | 1 | THERMAL STRAIN | A |
| 8 | 2 | 2 | 0 | 0 | 0 | THERMAL STRAIN | A |
| 9 | 3 | 3 | 1 | 0 | 0 | THERMAL STRAIN | A |
| 10 | 2 | 2 | 2 | 0 | 0 | THERMAL STRAIN | A |
| 11 | 5 | 5 | 4 | 0 | 0 | THERMAL STRAIN | A |
| 12 | 2 | 0 | 0 | 2 | 0 | THERMAL STRAIN | A |
| 13 | 4 | 0 | 0 | 4 | 0 | THERMAL STRAIN | A |
| 14 | 2 | 0 | 0 | 2 | 2 | THERMAL STRAIN | A |
| 15 | 4 | 0 | 0 | 4 | 3 | THERMAL STRAIN | A |
| 16 | 0 | 0 | 0 | 0 | 0 | THERMAL STRAIN | B |
| 17 | 0 | 0 | 0 | 0 | 0 | THERMAL STRAIN | C |
| 18 | 0 | 0 | 0 | 0 | 0 | THERMAL STRAIN | D |
| 19 | 9 | 0 | 0 | 0 | 0 | THERMAL STRAIN | E |

**[Table 2]**

| | EVALUATION OF IRON LOSS | EVALUATION OF NOISE | |
|---|---|---|---|
| | W/kg | dBA | |
| 1 | 1.075 | 36.8 | INVENTIVE EXAMPLE |
| 2 | 1.084 | 36.0 | INVENTIVE EXAMPLE |
| 3 | 1.092 | 35.7 | INVENTIVE EXAMPLE |
| 4 | 1.052 | 35.6 | INVENTIVE EXAMPLE |
| 5 | 1.076 | 36.5 | INVENTIVE EXAMPLE |
| 6 | 1.072 | 36.4 | INVENTIVE EXAMPLE |
| 7 | 1.048 | 36.1 | INVENTIVE EXAMPLE |
| 8 | 1.062 | 35.6 | INVENTIVE EXAMPLE |
| 9 | 1.063 | 35.5 | INVENTIVE EXAMPLE |
| 10 | 1.060 | 35.5 | INVENTIVE EXAMPLE |
| 11 | 1.058 | 34.5 | INVENTIVE EXAMPLE |
| 12 | 1.065 | 35.6 | INVENTIVE EXAMPLE |
| 13 | 1.063 | 35.2 | INVENTIVE EXAMPLE |
| 14 | 1.063 | 35.4 | INVENTIVE EXAMPLE |
| 15 | 1.061 | 34.8 | INVENTIVE EXAMPLE |
| 16 | 1.051 | 39.0 | COMPARATIVE EXAMPLE |
| 17 | 1.140 | 37.2 | COMPARATIVE EXAMPLE |
| 18 | 1.183 | 34.8 | COMPARATIVE EXAMPLE |
| 19 | 1.195 | 34.5 | COMPARATIVE EXAMPLE |

In Examples No. 1 to No. 3, the number of imaginary lines VL1 where the standard deviation of the distances of magnetic domain control points was 1.25 mm or more and the average value of the spacing of magnetic domain walls was 600 µm or less was 1. In Examples No. 1 to No. 3, both evaluation results of iron loss and noise were acceptable. Herein, in Examples No. 1 to No. 3, although the number of imaginary lines VL1 where the maximum value of the spacing of magnetic domain walls was 1200 µm or less was 0, the number of imaginary lines VL1 where the average value of the spacing of magnetic domain walls was 600 µm or less was 1, and thus, the excellent characteristics were obtained. Also in Examples No. 4 and No. 8 to No. 11, the number of imaginary lines VL1 where the average value of the spacing of magnetic domain walls was 600 µm or less was 1 or more, and thus, the excellent characteristics were obtained as in Examples No. 1 to No. 3.

In Example No. 4, the number of imaginary lines VL1 where the standard deviation of the distances of magnetic domain control points was 1.25 mm or more and the average value of the spacing of magnetic domain walls was 500 µm or less was 1. In Example No. 4, both evaluation results of iron loss and noise were acceptable. In addition, the evaluation results of iron loss and noise of Example No. 4 were better than those of Examples No. 1 to No. 3.

In Example No. 5, the number of imaginary lines VL1 where the standard deviation of the distances of magnetic domain control points was 1.25 mm or more and the maximum value of the spacing of magnetic domain walls was 1200 µm or less was 1. In Example No. 5, both evaluation results of iron loss and noise were acceptable. Herein, in Example No. 5, although the number of imaginary lines VL1 where the average value of the spacing of magnetic domain walls was 600 µm or less was 0, the number of imaginary lines VL1 where the maximum value of the spacing of magnetic domain walls was 1200 µm or less was 1, and thus, the excellent characteristics were obtained. Also in Examples No. 7 and No. 12 to No. 15, the number of imaginary lines VL1 where the maximum value of the spacing of magnetic domain walls was 1200 µm or less was 1 or more, and thus, the excellent characteristics were obtained as in Example No. 5.

In Example No. 6, the number of imaginary lines VL1 where the standard deviation of the distances of magnetic domain control points was 1.25 mm or more and the average value of the spacing of magnetic domain walls was 500 µm or less was 1, and the number of imaginary lines VL1 where the maximum value of the spacing of magnetic domain walls was 1200 µm or less was 1. In Example No. 6, both evaluation results of iron loss and noise were acceptable.

In Example No. 7, the number of imaginary lines VL1 where the standard deviation of the distances of magnetic domain control points was 1.25 mm or more and the maximum value of the spacing of magnetic domain walls was 800 µm or less was 1. In Example No. 7, both evaluation results of iron loss and noise were acceptable. In addition, the evaluation result of iron loss of Example No. 7 was better than that of Example No. 5.

In Example No. 8, the number of imaginary lines VL1 where the standard deviation of the distances of magnetic domain control points was 1.25 mm or more and the average value of the spacing of magnetic domain walls was 600 µm or less was 2. In Example No. 8, both evaluation results of iron loss and noise were acceptable. In addition, the evaluation results of iron loss and noise of Example No. 8 were better than those of Examples No. 1 to No. 3.

In Example No. 9, the number of imaginary lines VL1 where the standard deviation of the distances of magnetic domain control points was 1.25 mm or more and the average value of the spacing of magnetic domain walls was 500 µm or less was 1. In Example No. 9, both evaluation results of iron loss and noise were acceptable. In addition, the evaluation results of iron loss and noise of Example No. 9 were better than those of Examples No. 1 to No. 3.

In Example No. 10, the number of imaginary lines VL1 where the standard deviation of the distances of magnetic domain control points was 1.25 mm or more and the average value of the spacing of magnetic domain walls was 500 µm or less was 2. In Example No. 10, both evaluation results of iron loss and noise were acceptable. In addition, the evaluation result of iron loss of Example No. 10 was much better than that of Example No. 8.

In Example No. 11, the number of imaginary lines VL1 where the standard deviation of the distances of magnetic domain control points was 1.25 mm or more and the average value of the spacing of magnetic domain walls was 500 µm or less was 4. In Example No. 11, both evaluation results of iron loss and noise were acceptable. In addition, the evaluation result of iron loss of Example No. 11 was much better than that of Example No. 10.

In Example No. 12, the number of imaginary lines VL1 where the standard deviation of the distances of magnetic domain control points was 1.25 mm or more and the maximum value of the spacing of magnetic domain walls was 1200 µm or less was 2. In Example No. 12, both evaluation results of iron loss and noise were acceptable. In addition, the evaluation results of iron loss and noise of Example No. 12 were much better than those of Example No. 5.

In Example No. 13, the number of imaginary lines VL1 where the standard deviation of the distances of magnetic domain control points was 1.25 mm or more and the maximum value of the spacing of magnetic domain walls was 1200 µm or less was 4. In Example No. 13, both evaluation results of iron loss and noise were acceptable. In addition, the evaluation result of iron loss of Example No. 13 was much better than that of Example No. 12.

In Example No. 14, the number of imaginary lines VL1 where the standard deviation of the distances of magnetic domain control points was 1.25 mm or more and the maximum value of the spacing of magnetic domain walls was 800 µm or less was 2. In Example No. 14, both evaluation results of iron loss and noise were acceptable. In addition, the evaluation result of iron loss of Example No. 14 was much better than that of Example No. 12.

In Example No. 15, the number of imaginary lines VL1 where the standard deviation of the distances of magnetic domain control points was 1.25 mm or more and the maximum value of the spacing of magnetic domain walls was 800 µm or less was 3. In Example No. 15, both evaluation results of iron loss and noise were acceptable. In addition, the evaluation result of iron loss of Example No. 15 was much better than that of Example No. 14.

On the other hand, in Examples No. 16, No. 17, and No. 18 which were not subjected to selective magnetic domain control treatment, the number of imaginary lines VL1 where the standard deviation of the distances of magnetic domain control points was 1.25 mm or more was 0. In these Examples, both evaluation results of iron loss and noise were unacceptable.

In Example No. 19, the magnetic domain control treatment line having an interval of 4 mm was formed only in a region within ±4 mm from the center of each crystal grain in the rolling direction RD. The radius of curvature of the steel sheet at the position where the grains were present during the final annealing was 250 mm. In Example No. 19, the imaginary lines VL1 where the standard deviation of the distances of magnetic domain control points VP was 1.25 mm or more could be set. However, in all of the imaginary lines VL1, the average value of the spacing of magnetic domain walls was more than 600 µm, and the maximum value of the spacing of magnetic domain walls was more than 1200 µm. In Example No. 19, although the evaluation result of noise was sufficient, the evaluation result of iron loss was insufficient. This is presumably because the magnetic domain control treatment line was not formed in areas where the magnetic domain control was needed.

### (Example 2)

The magnetic domain control treatment was carried out on the grain-oriented electrical steel sheet under the same conditions as in the above Example 1, except for the type of grain-oriented electrical steel sheet used as the original sheet. Specifically, a grain-oriented electrical steel sheet (grain-oriented electrical steel sheet having coarse grain size) of the same lot having a sheet thickness of 0.23 mm was used as the original sheet. In these grain-oriented electrical steel sheets, for instance, the average temperature rising rate in a range from 1000 to 1200°C was less than 5°C/h during temperature rising process of final annealing. The original sheet was subjected to a magnetic domain control treatment under various conditions shown in Table 3. The magnetic flux density, noise, and iron loss of the grain-oriented electrical steel sheets subjected to the magnetic domain control treatment obtained as a result were evaluated and are described in Table 4. In Table 4, values determined to be unacceptable are underlined.

The shapes of the magnetic domain control treatment lines were the same as in the above Example 1. The methods for evaluating the noise and iron loss were also the same as in the above Example 1. Notating the manufacturing results and evaluation results in the tables was the same as in the above Example 1.

The method for evaluating the magnetic flux density was as follows. The magnetic flux density was obtained by measuring using the Epstein method specified in JIS C 2550-1:2011. The magnetic flux density B₈ (T) in the rolling direction of the steel sheet was measured under the condition such that the steel sheet was excited at 800 A/m. The measured magnetic flux density are described in Table 4 as the evaluation result of magnetic flux density (unit: T) of the grain-oriented electrical steel sheet. An example in which the evaluation result of magnetic flux density was 1.935 T or more was determined to be an example in which the magnetic flux density was more excellent than that of the grain-oriented electrical steel sheet having the general grain size.

Although not shown in the tables, in any imaginary lines VL1 where the standard deviation of the distances of magnetic domain control points VP was 1.25 mm or more, a number of grain boundary points which were intersection points between the imaginary lines VL1 and grain boundaries was 2 or less.

**[Table 3]**

| | NUMBER OF VL1 WHERE STANDARD DEVIATION IS 2.50 mm OR MORE | NUMBER OF VL1 WHERE AVERAGE SPACING OF MAGNETIC DOMAIN WALLS IS 600 *µ*m OR LESS | NUMBER OF VL1 WHERE AVERAGE SPACING OF MAGNETIC DOMAIN WALLS IS 500 *µ*m OR LESS | NUMBER OF VL1 WHERE MAXIMUM SPACING OF MAGNETIC DOMAIN WALLS IS 1200 *µ*m OR LESS | NUMBER OF VL1 WHERE MAXIMUM SPACING OF MAGNETIC DOMAIN WALLS IS 800 *µ*m OR LESS | TYPE OF MAGNETIC DOMAIN CONTROL TREATMENT LINE | REMARKS |
|---|---|---|---|---|---|---|---|
| 20 | 1 | 1 | 0 | 0 | 0 | THERMAL STRAIN | A |
| 21 | 1 | 1 | 0 | 0 | 0 | MIXED | A |
| 22 | 1 | 1 | 0 | 0 | 0 | GROOVE | A |
| 23 | 1 | 1 | 1 | 0 | 0 | THERMAL STRAIN | A |
| 24 | 1 | 0 | 0 | 1 | 0 | THERMAL STRAIN | A |
| 25 | 1 | 1 | 0 | 1 | 0 | THERMAL STRAIN | A |
| 26 | 1 | 0 | 0 | 1 | 1 | THERMAL STRAIN | A |
| 27 | 2 | 2 | 0 | 0 | 0 | THERMAL STRAIN | A |
| 28 | 3 | 3 | 1 | 0 | 0 | THERMAL STRAIN | A |
| 29 | 2 | 2 | 2 | 0 | 0 | THERMAL STRAIN | A |
| 30 | 4 | 4 | 3 | 0 | 0 | THERMAL STRAIN | A |
| 31 | 2 | 0 | 0 | 2 | 0 | THERMAL STRAIN | A |
| 32 | 4 | 0 | 0 | 4 | 0 | THERMAL STRAIN | A |
| 33 | 2 | 0 | 0 | 2 | 2 | THERMAL STRAIN | A |
| 34 | 3 | 0 | 0 | 3 | 3 | THERMAL STRAIN | A |
| 35 | 0 | 0 | 0 | 0 | 0 | THERMAL STRAIN | B |
| 36 | 0 | 0 | 0 | 0 | 0 | THERMAL STRAIN | C |
| 37 | 0 | 0 | 0 | 0 | 0 | THERMAL STRAIN | D |
| 38 | 9 | 0 | 0 | 0 | 0 | THERMAL STRAIN | E |

**[Table 4]**

| | EVALUATION OF MAGNETIC FLUX DENSITY | EVALUATION OF IRON LOSS | EVALUATION OF NOISE | |
|---|---|---|---|---|
| | T | W/kg | dBA | |
| 20 | 1.935 | 1.031 | 32.9 | INVENTIVE EXAMPLE |
| 21 | 1.938 | 1.035 | 32.5 | INVENTIVE EXAMPLE |
| 22 | 1.936 | 1.039 | 32.2 | INVENTIVE EXAMPLE |
| 23 | 1.937 | 1.028 | 32.0 | INVENTIVE EXAMPLE |
| 24 | 1.941 | 1.022 | 33.5 | INVENTIVE EXAMPLE |
| 25 | 1.936 | 1.023 | 32.6 | INVENTIVE EXAMPLE |
| 26 | 1.935 | 1.011 | 33.2 | INVENTIVE EXAMPLE |
| 27 | 1.942 | 1.018 | 30.6 | INVENTIVE EXAMPLE |
| 28 | 1.937 | 1.016 | 30.2 | INVENTIVE EXAMPLE |
| 29 | 1.939 | 1.014 | 29.8 | INVENTIVE EXAMPLE |
| 30 | 1.941 | 1.011 | 29.5 | INVENTIVE EXAMPLE |
| 31 | 1.936 | 1.008 | 31.8 | INVENTIVE EXAMPLE |
| 32 | 1.940 | 1.007 | 31.6 | INVENTIVE EXAMPLE |
| 33 | 1.937 | 1.003 | 31.4 | INVENTIVE EXAMPLE |
| 34 | 1.941 | 1.001 | 31.1 | INVENTIVE EXAMPLE |
| 35 | 1.935 | 1.034 | 38.7 | COMPARATIVE EXAMPLE |
| 36 | 1.937 | 1.117 | 37.0 | COMPARATIVE EXAMPLE |
| 37 | 1.940 | 1.146 | 34.5 | COMPARATIVE EXAMPLE |
| 38 | 1.939 | 1.159 | 34.2 | COMPARATIVE EXAMPLE |

In the examples in which at least one imaginary line VL1 where the standard deviation of the distances of magnetic domain control points VP was 2.50 mm or more and where the average value of the spacing of magnetic domain walls was 600 µm or less or the maximum value of the spacing of magnetic domain walls was 1200 µm or less when measured along the imaginary line VL1 could be set, all of the evaluation results of the magnetic flux density, the iron loss, and the noise were sufficient. In general, the steel sheet having a coarse grain size has excellent magnetic flux density, the noise characteristics tend to deteriorate when the conventional magnetic domain control treatment is performed. On the other hand, in Examples No. 20 to No. 34 shown in Table 3 and Table 4, the magnetic domain control treatment line was formed on the basis of the distribution of the spacing of magnetic domain walls, and thus, all of the evaluation results of the magnetic flux density, the iron loss, and the noise were sufficient as explained above.

In the same way, in Examples No. 20 to No. 34 where the number of grain boundary points which were the intersection points VP of the grain boundaries in the imaginary line VL1 where the standard deviation of the distances of magnetic domain control points was 1.25 mm or more was 2 or less, all of the evaluation results of the magnetic flux density, the iron loss, and the noise were sufficient as explained above.

On the other hand, in Examples No. 35, No. 36, and No. 37 which were not subjected to selective magnetic domain control treatment, the number of imaginary lines VL1 where the standard deviation of the distances of magnetic domain control points VP was 2.50 mm or more was 0. Moreover, in all of the imaginary lines VL1, the average value of the spacing of magnetic domain walls was more than 600 µm, and the maximum value of the spacing of magnetic domain walls was more than 1200 µm. In these Examples, at least one of evaluation results of iron loss or noise was unacceptable.

In Example No. 38, the magnetic domain control treatment line having an interval of 4 mm was formed only in a region within ±4 mm from the center of each crystal grain in the rolling direction RD. The radius of curvature of the steel sheet at the position where the grains were present during the final annealing was 250 mm. In Example No. 38, the imaginary lines VL1 where the standard deviation of the distances of magnetic domain control points VP was 2.50 mm or more could be set. However, in all of the imaginary lines VL1, the average value of the spacing of magnetic domain walls was more than 600 µm, and the maximum value of the spacing of magnetic domain walls was more than 1200 µm. In Example No. 38, although the evaluation result of noise was sufficient, the evaluation result of iron loss was insufficient. This is presumably because the magnetic domain control treatment line was not formed in areas where the magnetic domain control was needed.

### INDUSTRIAL APPLICABILITY

According to the present disclosure, it is possible to provide a grain-oriented electrical steel sheet capable of achieving both iron loss reduction and noise reduction, and a method for manufacturing the same. Accordingly, the present invention has significant industrial applicability.

### REFERENCE SIGNS LIST

- 1: Grain-oriented electrical steel sheet
- 11: Magnetic domain control treatment line
- RD: Rolling direction
- TD: Transverse direction
- ND: Rolled surface normal direction
- VL1: First imaginary line
- VP: Magnetic domain control point
- VL2: Second imaginary line
- X: Region where no magnetic domain control treatment line is formed
- 2: Original sheet
- 21: Magnetic domain control treatment region
- 22: Non-magnetic domain control treatment region
- 30: Image acquisition device
- 31: Light source unit
- 33: MO sensor
- 35: Image sensor
- 37: Signal processing unit
- 40: Analysis device
- 41: Calculation unit
- 43: Memory
- 45: Display unit
- 47: Input unit
- 49: Communication I/F
- 500: Laser irradiation device
- 501: Polygon mirror
- 503: light source device
- 505: Collimator
- 507: Condensing lens
- 509: Motor
- 511: Sensor
- 513: Control unit
- 515: Sheet passing device

## Claims

1. A grain-oriented electrical steel sheet having plural magnetic domain control treatment lines on a surface thereof, wherein,
when an evaluation region with a square shape where a length of each side is 50 mm and a side is parallel to a rolling direction of the grain-oriented electrical steel sheet is determined in the grain-oriented electrical steel sheet and when imaginary lines parallel to the rolling direction with a length of 50 mm are set with a spacing of 5 mm in the evaluation region,
in at least one of the imaginary lines, a standard deviation of distances of magnetic domain control points which are intersection points between the imaginary lines and the magnetic domain control treatment lines is 1.25 mm or more, and an average value of spacing of magnetic domain walls measured along the imaginary line is 600 µm or less.

2. The grain-oriented electrical steel sheet according to claim 1, wherein,
in the imaginary lines where the standard deviation of the distances of the magnetic domain control points is 1.25 mm or more, the average value of the spacing of magnetic domain walls is 500 µm or less.

3. A grain-oriented electrical steel sheet having plural magnetic domain control treatment lines on a surface thereof, wherein,
when an evaluation region with a square shape where a length of each side is 50 mm and a side is parallel to a rolling direction of the grain-oriented electrical steel sheet is determined in the grain-oriented electrical steel sheet and when imaginary lines parallel to the rolling direction with a length of 50 mm are set with a spacing of 5 mm in the evaluation region,
in at least one of the imaginary lines, a standard deviation of distances of magnetic domain control points which are intersection points between the imaginary lines and the magnetic domain control treatment lines is 1.25 mm or more, and a maximum value of spacing of magnetic domain walls measured along the imaginary line is 1200 µm or less.

4. The grain-oriented electrical steel sheet according to claim 3, wherein,
in the imaginary lines where the standard deviation of the distances of the magnetic domain control points is 1.25 mm or more, the maximum value of the spacing of magnetic domain walls is 800 µm or less.

5. The grain-oriented electrical steel sheet according to claim 1, wherein,
in each of two or more of the imaginary lines, the standard deviation of the distances of the magnetic domain control points is 1.25 mm or more, and the average value of the spacing of magnetic domain walls is 600 µm or less.

6. The grain-oriented electrical steel sheet according to claim 5, wherein,
in each of two or more of the imaginary lines where the standard deviation of the distances of the magnetic domain control points is 1.25 mm or more, the average value of the spacing of magnetic domain walls is 500 µm or less.

7. The grain-oriented electrical steel sheet according to claim 1, wherein,
in at least one of the imaginary lines, the standard deviation of the distances of the magnetic domain control points which are intersection points between the imaginary lines and the magnetic domain control treatment lines is 2.50 mm or more, and the average value of the spacing of magnetic domain walls measured along the imaginary line is 600 µm or less.

8. The grain-oriented electrical steel sheet according to claim 7, wherein,
in the imaginary lines where the standard deviation of the distances of the magnetic domain control points is 2.50 mm or more, the average value of the spacing of magnetic domain walls is 500 µm or less.

9. The grain-oriented electrical steel sheet according to claim 1, wherein,
in at least one of the imaginary lines in the imaginary lines where the standard deviation of the distances of the magnetic domain control points is 1.25 mm or more, a number of grain boundary points which are intersection points between the imaginary lines and grain boundaries is 2 points or less.

10. The grain-oriented electrical steel sheet according to claim 9, wherein,
in each of two or more of the imaginary lines, the number of grain boundary points is 2 points or less.

11. The grain-oriented electrical steel sheet according to claim 3, wherein,
in each of two or more of the imaginary lines, the standard deviation of the distances of the magnetic domain control points is 1.25 mm or more, and the maximum value of the spacing of magnetic domain walls is 1200 µm or less.

12. The grain-oriented electrical steel sheet according to claim 11, wherein,
in each of two or more of the imaginary lines where the standard deviation of the distances of the magnetic domain control points is 1.25 mm or more, the maximum value of the spacing of magnetic domain walls is 800 µm or less.

13. The grain-oriented electrical steel sheet according to claim 3, wherein,
in at least one of the imaginary lines, the standard deviation of the distances of the magnetic domain control points which are intersection points between the imaginary lines and the magnetic domain control treatment lines is 2.50 mm or more, and the maximum value of the spacing of magnetic domain walls measured along the imaginary line is 1200 µm or less.

14. The grain-oriented electrical steel sheet according to claim 13, wherein,
in the imaginary lines where the standard deviation of the distances of the magnetic domain control points is 2.50 mm or more, the maximum value of the spacing of magnetic domain walls is 800 µm or less.

15. The grain-oriented electrical steel sheet according to claim 3, wherein,
in at least one of the imaginary lines in the imaginary lines where the standard deviation of the distances of the magnetic domain control points is 1.25 mm or more, a number of grain boundary points which are intersection points between the imaginary lines and grain boundaries is 2 points or less.

16. The grain-oriented electrical steel sheet according to claim 15, wherein,
in each of two or more of the imaginary lines, the number of grain boundary points is 2 points or less.

17. The grain-oriented electrical steel sheet according to any one of claims 1 to 16, wherein the magnetic domain control treatment lines are thermal strain.

18. The grain-oriented electrical steel sheet according to any one of claims 1 to 16, wherein the magnetic domain control treatment lines are grooves.

19. The grain-oriented electrical steel sheet according to any one of claims 1 to 16, wherein, in at least one of the imaginary lines, the standard deviation of the distances is less than 1.25mm.

20. A method for manufacturing a grain-oriented electrical steel sheet comprising:
a step of acquiring a magnetic domain image of an original sheet of a grain-oriented electrical steel sheet;
a step of determining a magnetic domain control treatment region based on a distribution of spacing of magnetic domain walls in the magnetic domain image; and
a step of applying a magnetic domain control treatment to the magnetic domain control treatment region determined based on the distribution of the spacing of magnetic domain walls; wherein,
when an evaluation region with a square shape where a length of each side is 50 mm and a side is parallel to a rolling direction of the grain-oriented electrical steel sheet is determined in the grain-oriented electrical steel sheet and when imaginary lines parallel to the rolling direction with a length of 50 mm are set with a spacing of 5 mm in the evaluation region,
in at least one of the imaginary lines, a standard deviation of distances of magnetic domain control points which are intersection points between the imaginary lines and the magnetic domain control treatment lines formed by the magnetic domain control treatment is controlled to 1.25 mm or more.

21. The method for manufacturing the grain-oriented electrical steel sheet according to claim 20, wherein a region where the spacing of magnetic domain walls is a predetermined value or more is set as the magnetic domain control treatment region.

22. The method for manufacturing a grain-oriented electrical steel sheet according to claim 20 or 21, wherein a distribution of the spacing of magnetic domain walls is derived from the magnetic domain image using a two-dimensional Fourier transform.

23. The method for manufacturing a grain-oriented electrical steel sheet according to claim 20 or 21, wherein the magnetic domain control treatment is applied by irradiation with a laser or an electron beam.
